



US005885700A

**United States Patent** [19]**Weldon et al.****Patent Number:** **5,885,700****Date of Patent:** **Mar. 23, 1999**[54] **THERMOPLASTIC LENS BLOCKING MATERIAL**

[75] Inventors: **James A. Weldon**, Eagan; **Michael Govek**, Lakeville; **Carole Sedlock**, Minneapolis; **John H. Ko**, Woodbury, all of Minn.

[73] Assignee: **Minnesota Mining and Manufacturing Company**, St. Paul, Minn.

[21] Appl. No.: **818,266**

[22] Filed: **Mar. 17, 1997**

**Related U.S. Application Data**

[63] Continuation-in-part of Ser. No. 713,344, Sep. 13, 1996, Pat. No. 5,754,269.

[60] Provisional application No. 60/003,918 Sep. 18, 1995.

[51] **Int. Cl.**<sup>6</sup> ..... **B32B 7/02**

[52] **U.S. Cl.** ..... **428/212; 428/217; 428/424.8; 428/426; 451/390; 351/159**

[58] **Field of Search** ..... **428/212, 217, 428/411.1, 424.8, 426; 451/390; 351/159**

[56] **References Cited****U.S. PATENT DOCUMENTS**

|            |         |                  |       |            |
|------------|---------|------------------|-------|------------|
| Re. 24,906 | 12/1960 | Ulrich           | ..... | 206/59     |
| 3,382,202  | 5/1968  | Forrester et al. | ..... | 260/32.6   |
| 3,468,366  | 9/1969  | Suddarth         | ..... | 164/332    |
| 3,512,310  | 5/1970  | Rudd et al.      | ..... | 51/277     |
| 3,651,014  | 3/1972  | Witsiepe         | ..... | 260/75 R   |
| 3,786,116  | 1/1974  | Milkovich et al. | ..... | 260/885    |
| 3,911,185  | 10/1975 | Wright, Jr.      | ..... | 428/97     |
| 3,914,489  | 10/1975 | Smedberg         | ..... | 428/97     |
| 3,926,878  | 12/1975 | Shimizu et al.   | ..... | 260/27 EV  |
| 3,944,695  | 3/1976  | Kosaka et al.    | ..... | 428/200    |
| 3,996,701  | 12/1976 | Ramirez et al.   | ..... | 51/216 LP  |
| 4,025,694  | 5/1977  | Pletcher         | ..... | 428/480    |
| 4,059,715  | 11/1977 | Pletcher         | ..... | 428/349    |
| 4,066,600  | 1/1978  | Pletcher et al.  | ..... | 260/30.6 R |

(List continued on next page.)

**FOREIGN PATENT DOCUMENTS**

|              |         |                      |
|--------------|---------|----------------------|
| 0 359 135    | 3/1990  | European Pat. Off. . |
| 0 443 269 B1 | 10/1993 | European Pat. Off. . |
| 0 642 039 A2 | 3/1995  | European Pat. Off. . |
| Sho 46-21120 | 6/1971  | Japan .              |
| Hei.4-146983 | 5/1992  | Japan .              |
| 2 017 546    | 10/1979 | United Kingdom .     |
| WO 92/08614  | 5/1992  | WIPO .               |
| WO 93/07228  | 4/1993  | WIPO .               |
| WO 97/10923  | 7/1996  | WIPO .               |
| WO 97/10924  | 9/1996  | WIPO .               |

**OTHER PUBLICATIONS**

“Step One: Your First Step in Surface Preparation”, Lab Talk, Jan./Feb. 1994, pp. 6, 8, 18.

Gerber Optical, Inc. product literature, copyright Nov. 17, 1993.

Fast Grind® product literature, Super Systems, copyright unknown.

Advanced Blocking System product literature, Optical Works Corp., copyright unknown (2 sheets).

International Search Report for PCT/US/98/00803.

International Search Report for PCT/US/98/03715.

*Primary Examiner*—Elizabeth Evans  
*Attorney, Agent, or Firm*—F. Andrew Ubel

[57] **ABSTRACT**

The present invention provides thermoplastic ophthalmic lens blocking compositions that have many advantages over traditional metal alloy materials. Preferred compositions comprise a blend of (i) a hydrocarbon resin, preferably an aromatic hydrocarbon resin; (ii) a side chain crystallizable hydrocarbon polymer or copolymer; and (iii) optionally an modifier or mixture of modifiers, preferably straight chain alcohols. The composition may also comprise one or more modifiers, fillers or heat absorbing materials. In one embodiment, the composition is used to fill the cavity between a preformed lens block and a lens. In another embodiment the composition is used to form a lens block. Methods of holding a lens blank are taught. Tapes that provide a receptive surface against which the composition may be adhered are disclosed.

**20 Claims, 4 Drawing Sheets**

## U.S. PATENT DOCUMENTS

|           |         |                    |       |             |           |         |                  |       |         |
|-----------|---------|--------------------|-------|-------------|-----------|---------|------------------|-------|---------|
| 4,173,506 | 11/1979 | Pletcher           | ..... | 156/309     | 4,740,245 | 4/1988  | Futami et al.    | ..... | 106/35  |
| 4,182,829 | 1/1980  | Walkowiak et al.   | ..... | 528/75      | 4,768,951 | 9/1988  | Abiru et al.     | ..... | 433/48  |
| 4,235,761 | 11/1980 | Koenig             | ..... | 260/28.5 AV | 4,833,179 | 5/1989  | Young et al.     | ..... | 522/183 |
| 4,280,939 | 7/1981  | Johnson            | ..... | 260/23 AR   | 4,847,137 | 7/1989  | Kellen et al.    | ..... | 428/195 |
| 4,287,013 | 9/1981  | Ronning            | ..... | 156/242     | 4,952,650 | 8/1990  | Young et al.     | ..... | 526/194 |
| 4,327,013 | 4/1982  | Peters             | ..... | 524/538     | 5,026,278 | 6/1991  | Oxman et al.     | ..... | 433/41  |
| 4,328,060 | 5/1982  | Tusinski et al.    | ..... | 156/344     | 5,040,976 | 8/1991  | Ubel, III et al. | ..... | 433/41  |
| 4,352,749 | 10/1982 | Nakabayashi et al. | ..... | 525/149     | 5,066,231 | 11/1991 | Oxman et al.     | ..... | 433/214 |
| 4,361,538 | 11/1982 | Dicoi et al.       | ..... | 422/62      | 5,096,969 | 3/1992  | Payne et al.     | ..... | 525/222 |
| 4,404,299 | 9/1983  | Decroix            | ..... | 524/77      | 5,183,705 | 2/1993  | Birkholz et al.  | ..... | 428/343 |
| 4,430,479 | 2/1984  | Merton et al.      | ..... | 525/127     | 5,194,500 | 3/1993  | Chin et al.      | ..... | 525/97  |
| 4,552,906 | 11/1985 | Podszun et al.     | ..... | 523/115     | 5,326,413 | 7/1994  | Esemplare et al. | ..... | 156/154 |
| 4,569,342 | 2/1986  | von Nostitz        | ..... | 128/136     | 5,403,188 | 4/1995  | Oxman et al.     | ..... | 433/218 |
| 4,659,786 | 4/1987  | Kawakami et al.    | ..... | 525/415     | 5,415,544 | 5/1995  | Oxman et al.     | ..... | 433/48  |
| 4,678,836 | 7/1987  | McKinney et al.    | ..... | 525/221     | 5,505,654 | 4/1996  | Wood et al.      | ..... | 451/6   |
| 4,737,559 | 4/1988  | Kellen et al.      | ..... | 526/291     | 5,520,568 | 5/1996  | Craighead et al. | ..... | 451/42  |
|           |         |                    |       |             | 5,721,644 | 2/1998  | Murray et al.    | ..... | 359/819 |



*Fig. 1*



*Fig. 2*



*Fig. 3*



*Fig. 4a*



*Fig. 4b*



*Fig. 4c*



*Fig. 5a*



*Fig. 5b*



*Fig. 6a*



*Fig. 6b*



*Fig. 7a*



*Fig. 7b*



*Fig. 8a*



*Fig. 8b*



*Fig. 8c*



*Fig. 8d*

**Fig. 8e****Fig. 8f****Fig. 8g****Fig. 9e****Fig. 9f****Fig. 9g****Fig. 10e****Fig. 10f****Fig. 10g**

## THERMOPLASTIC LENS BLOCKING MATERIAL

This application is a continuation-in-part of U.S. patent application Ser. No. 08/713,344, filed Sep. 13, 1996 now U.S. Pat. No. 5,754,269 issued May 19, 1998, which claims priority to U.S. provisional application Ser. No. 60/003,918, filed Sep. 18, 1995.

### FIELD

The present invention relates generally to a thermoplastic blocking composition for use in forming or attaching a lens block to an ophthalmic lens blank or a lens blank coating or tape and to preformed base blocks and lens blank tapes used with the blocking composition. The present invention also relates generally to methods of forming or attaching a lens block to an ophthalmic lens blank thereby facilitating the use of conventional machining, grinding and processing equipment to generate the ophthalmic lens.

### BACKGROUND

A number of different methods have been used to hold a lens in place during the surfacing process. The method most commonly used at present makes use of a low-melting-temperature metal alloy to form or attach a "block" to the semifinished surface of a lens "blank." This procedure is often referred to as "lens blocking."

A common low-melting-temperature alloy comprises bismuth, tin, lead, cadmium, indium, and antimony. When these elements are combined correctly, the alloy melts at a temperature considerably lower than any one of its component elements would melt by itself. The alloy will neither cause a plastic lens to melt nor a glass lens to crack. For example, one alloy that melts at 47° C. is made from the following combination of metals: 45% bismuth; 23% lead; 8% tin; 5% cadmium; and 19% indium. This alloy will work for either plastic or glass lenses. In general, a higher melting alloy (e.g., one which melts at 70° C.) will generally only work for glass lenses.

Unfortunately, many of the present metal alloy materials pose significant environmental and health hazards. For example, lead, a common ingredient in many alloys, is considered to be a strong protoplasmic poison which can be introduced into the body through ingestion, inhalation and skin absorption. Similarly, cadmium may also pose significant health hazards. These hazards are particularly acute since many of the procedures used in the ophthalmic laboratory may cause fumes and/or dust particles of these metals to be released to the air, thereby creating environmental and health hazards for those formulating these alloys or those working with them.

A "blocker" is a piece of equipment employed for the purpose of lens blocking. Blockers that use metal alloy either inject molten alloy between the semifinished lens and a preformed block, or mold a block fully and completely from the alloy material. Both types of blockers have a melting pot that is thermostatically regulated, and a heated feeding tube.

Ideally, for plastic lenses, the alloy temperature is kept just above its melting point until it fills in the cavity between the lens and lens block. For example, the 47° C. alloy used for plastic, polycarbonate and polyurethane lenses should preferably be kept at 52° C., or even lower if possible. For glass lenses the alloy temperature may be maintained at higher temperatures (e.g., about 77° C.).

Once on the lens, the alloy should be cooled as rapidly as possible. In addition to saving time, rapid cooling of the

alloy helps prevent the formation of aberrations or indentations on the surface of the lens. However, it is also important that the alloy be allowed to cool fully before generating the lens. If a lens is generated too soon after blocking, the alloy may not have cooled evenly, thereby producing surface distortion or waviness or the lens may become dislodged from the blank.

There are two convenient ways used to harden the alloy quickly. The first is to circulate cold running water or a coolant through a water or "chill" ring, which fits around the lens block. This causes the lens block and alloy to chill, "freezing" the alloy. The second method is to chill the block (e.g., in a refrigerator) before it is placed on the blocker.

A tape or other lens coating is often used when surfacing lenses: (1) to prevent the lenses from being scratched; (2) to serve as a heat shield (e.g., to protect a plastic lens from warpage caused by the heat of the alloy); (3) to achieve better or enhanced alloy adherence; and (4) to eliminate the step of cleaning the lens after surfacing. The cleanest and most common method for protecting lens surfaces and holding the block securely is the use of a surface tape. Tapes for this purpose were developed by the 3M Company and may be applied by placing the lens in a small chamber, stretching the tape over the chamber, and applying a partial vacuum. The lens moves up to the tape and the tape is pulled down over the lens surface. Alternatively, lens coatings, available in brush-on and spray applications, may be applied to the convex side of the lens.

Blocks used for glass lenses ("glass blocks" or "glass-lens blocks") are generally about 43 mm in diameter. They do not need to be large, since their purpose is purely to hold the lens during generating. Blocks used for plastic lenses ("plastic-lens blocks") must not only hold the lens in place, they must also keep it from flexing (bending) during generating, fining, and polishing. For that reason, plastic-lens blocks are generally considerably larger than glass-lens blocks. Since blocks for plastic lenses should be made as large as possible for each grinding situation, they are available in a variety of sizes ranging from approximately 55 to 68 mm. Generally, the largest block that can be used on a given semifinished lens blank is chosen. It should be understood that "glass-lens blocks" are generally made from steel, not glass. They are normally used for blocking glass lenses. Neither are "plastic-lens blocks" made exclusively from plastic. Such blocks are normally made from aluminum.

When a lens has been blocked using a metal alloy, it can be deblocked through shock deblocking or hot-water deblocking.

Shock deblocking of plastic lenses is done with a ring that is placed around the outside of the lens block on the front surface of the lens. It is deeper than the block, so when the lens and block are turned block side down, the ring may be struck against a flat surface. The block drops off the lens from the shock.

Hot-water deblocking is a commonly used technique that utilizes a hot-water bath. The temperature of the water is kept below the boiling point. The blocked lenses are placed on a rack, which is lowered into the water. With the lens under water, the alloy begins to melt and drips to the bottom of the tank. There is a valve at the bottom of the tank through which the liquid alloy can be drained off from time to time. After deblocking, the blocks and lenses are removed from the rack, the surface tape removed, and the lenses cleaned.

Attempts have been made to use less toxic materials in place of the toxic metal alloy. For example, materials comprising low molecular weight thermoplastic polymers

and resins have been tried. Unfortunately, some of these compositions exhibit generally poor physical properties (e.g., they are relatively brittle and of little cohesive or tensile strength). Others are very soft and waxy (or become soft and waxy during use), and are prone to flexing which could cause lens distortion during processing. In addition, some of these compositions are also very tacky and messy to work with and do not directly adhere well to glass lenses. Cleaning of these tacky compositions from lens blanks can be very time consuming and significantly increase the cost of the lens processing operation. Also, current wax compositions tend to be heat sensitive at temperatures encountered during normal processing conditions (e.g., grinding and polishing). Materials that are sensitive to normal operating temperatures (e.g., those materials that soften significantly at those temperatures) are undesirable for use in this application. Also, some of the wax based materials are not recommended for use in this application. Also, some of the wax based materials are not recommended for use with glass lenses or cannot be used in the presence of petroleum based lubricants.

### SUMMARY

We have discovered blocking compositions that have many advantages over traditional metal alloy materials. For example, the lens blocking compositions of the present invention are non-toxic, environmentally safe, and preferably biodegradable. The materials preferably can be used with existing processing equipment and may be recycled.

In one embodiment an ophthalmic lens block is provided that comprises a solidified mass of a thermoplastic blocking composition. The blocking composition may comprise, for example, a homopolymer or copolymer of epsilon-caprolactone. The composition may alternatively comprise, for example, a blend of (i) a hydrocarbon resin, preferably an aromatic hydrocarbon resin; (ii) a side chain crystallizable hydrocarbon polymer or copolymer; and (iii) optionally a modifier or mixture of modifiers, preferably straight chain alcohols. The blocking composition preferably has a number average molecular weight of at least 1,000, a mean bending modulus of at least 69 MPa at 21° C., or a mean flexural strength of at least 1 MPa at 21° C.

The composition is solid at 21° C. and has a sufficiently low melting or softening point such that the composition may be placed adjacent to an ophthalmic lens blank while at its melting or softening point without damaging the lens blank. The composition also has sufficient adhesion to a lens blank or to a lens blank coating or tape to hold an ophthalmic lens during a generating procedure. Ophthalmic lens blocking kits are provided that comprise the thermoplastic blocking composition and optionally a lens blank tape or coating and/or a preformed base block. Preferred preformed base blocks comprise a front portion that has a negatively tapered peripheral edge. The preferred preformed base block readily retains the thermoplastic blocking composition, yet can be easily separated from it after use. Preferred lens blank tapes are conformable and comprise a polymer backing that has both polar and non-polar moieties or an overall intermediate polar nature. By adjusting the ratio of polar and non-polar moieties of the surface of the tape, the adhesion to a thermoplastic blocking composition can be adjusted.

In another embodiment, a method of holding an ophthalmic lens blank is provided, comprising the steps of: providing a lens blocking composition as described above; heating the lens blocking composition to its melting or softening point; providing a blocking material receiving

cavity against the lens blank; forming the ophthalmic lens blocking composition into the receiving cavity; and allowing the composition to solidify. Alternatively, a method of holding an ophthalmic lens blank is provided, comprising the steps of: providing an ophthalmic lens block comprising a solidified mass of a thermoplastic blocking composition, and preferably comprising a heat absorbing material; heating the surface of the lens blocking composition to its melting or softening point; positioning a lens blank against the softened surface of the lens blocking composition; and allowing the composition to resolidify.

### RELATED APPLICATIONS

Of related interest is the following U.S. Provisional Patent Application, filed on Sep. 18, 1995 by the assignee of this invention: Lens Blank Surface Protection Film—Ser. No. 60/004,120; and U.S. Patent Application, filed on Nov. 17, 1995 by the assignee of this invention: Lens Blank Surface Protection Film—Ser. No. 08/560,315, pending, which are herein incorporated by reference. Also of related interest are the following pending U.S. applications Ser. No. 08,710,238, now U.S. Pat. No. 5,763,075 issued Jun. 9, 1998, Ser. No. 08/713,901, pending, Ser. No. 08/713,345, pending, and Ser. No. 08/713,322, pending, which are herein incorporated by reference.

### BRIEF DESCRIPTION OF THE DRAWINGS

This invention will be better understood when taken in conjunction with the drawings wherein:

FIG. 1 is a perspective view of an ophthalmic lens blank and a lens block;

FIG. 2 is a side view of an ophthalmic lens blank and a lens block, wherein the ophthalmic lens blank and a lens block are attached using a lens blocking composition of the present invention;

FIG. 3 is an end view of the ophthalmic lens blank and lens block of FIG. 2;

FIGS. 4a and 4b are side and end views of an ophthalmic lens blank and a lens block formed from a lens blocking composition of the present invention, FIG. 4c is a side view of an ophthalmic lens blank and a mold into which a lens blocking composition of the present invention may be injected to form a lens block;

FIGS. 5a and 5b are side and end views of an alternative ophthalmic lens blank and a lens block formed from a lens blocking composition of the present invention;

FIGS. 6a and 6b are side and end views of an alternative ophthalmic lens blank and a lens block formed in part from a lens blocking composition of the present invention and using a preformed base block;

FIGS. 7a and 7b are side and end views of an alternative ophthalmic lens blank and a lens block formed in part from a lens blocking composition of the present invention and using a preformed base block;

FIG. 8a is a side view of an ophthalmic lens blank and a lens block formed in part from a lens blocking composition of the present invention and using a preformed base block, FIG. 8b is a side view of the ophthalmic lens blank and block of FIG. 8a, further showing a cross-section of a chill ring mold, FIG. 8c is a cross-sectional view of the block of FIGS. 8a and 8b;

FIG. 8d is a cross sectional view of a block similar to the block depicted in FIGS. 8a and 8b, but having an alternative location for the filling gate;

FIGS. 8e to 8g are side and end views of the preformed base block of FIG. 8c;

FIGS. 9e to 9g are side and end views of an alternative preformed base block having a scalloped outer edge; and

FIGS. 10e to 10g are side and end views of a further alternative preformed base block having a keyed outer edge.

This invention utilizes certain principles and/or concepts as are set forth in the claims appended to this specification. Those skilled in the lens generating arts to which this invention pertains will realize that these principles and/or concepts are capable of being illustrated in a variety of embodiments which may differ from the exact embodiments utilized for illustrative purposes in this specification. For these reasons, the invention described in this specification is not to be construed as being limited to only the illustrative embodiments but is only to be construed in view of the appended claims.

#### DEFINITIONS

Unless otherwise specified, the term "molecular weight" in this specification refers to "weight average molecular weight." ( $M_w = \sum_i N_i M_i^2 / \sum_i N_i M_i$ ) Although weight average molecular weight ( $M_w$ ) can be determined in a variety of ways, with some differences in result depending upon the method employed, it is convenient to employ gel permeation chromatography. Standard sample preparation techniques should be observed. Molecular weight values reported by commercial suppliers of various materials are not always represented to be weight average molecular weight. The reported molecular weight is often presented in order to identify the particular material.

As used herein, the term "number average molecular weight" ( $M_n$ ) refers to the total weight of all the molecules in a polymer sample divided by the total number of moles present. ( $M_n = \sum_i N_i M_i / \sum_i N_i$ ) Although number average molecular weight can be determined in a variety of ways, with some differences in result depending upon the method employed, it is convenient to employ gel permeation chromatography.

As used herein, the term "Z average molecular weight" ( $M_z$ ) refers to a weighted average molecular weight defined by the equation  $M_z = \sum_i N_i M_i^3 / \sum_i N_i M_i^2$ . Although Z average molecular weight can be determined in a variety of ways, with some differences in result depending upon the method employed, it is convenient to employ gel permeation chromatography.

As used herein, the term "polydispersity" refers to the ratio of a materials' "weight average molecular weight" divided by its "number average molecular weight." ( $M_w/M_n$ )

As used herein, the term "melting or softening point" refers to the temperature at which a material has changed from its cool state to its warm state and is capable of being shaped to conform to a lens blank.

As used herein, a "lens block" refers to the entire three-dimensional apparatus that is attached to the lens blank and used to "handle" the lens blank during processing. This term includes any optional preformed base block and the thermoplastic blocking composition that attaches the preformed base block to the lens. This term does not include the lens itself or any lens surface protection tape or coating that is applied to the lens prior to blocking.

#### DETAILED DESCRIPTION

A variety of materials can be used in the ophthalmic lens blocking compositions of the present invention. The materials described herein provide a blocking composition that has many advantages over traditional metal alloys. For

example, the materials are non-toxic, environmentally safe, and preferably biodegradable. The materials preferably can be used with existing processing equipment and may be recycled.

Preferred compositions comprise a thermoplastic material, selection of which should be based in part on the desired end use for the composition (e.g., the type of lens being blocked, whether the composition is being used to form a block or attach a preformed block, etc.) and the desired properties of the composition in the molten or softened ("warm") state and solid or hard ("cool") state.

The warm state is characterized by appreciable mass flow of the blocking composition under moderate pressure at some temperature between above room temperature (preferably above about 35° C.) and the maximum temperature that can be safely tolerated by the lens blank against which the composition is formed or applied (e.g., for a thermoplastic material preferably below about 85° C., more preferably below about 75° C.). Notably, preferred thermoplastic materials of the present invention have a sufficiently high heat capacity that a temperature of 85° C. can be tolerated. In contrast, metal alloys heated to 85° C. might cause a plastic lens to melt or warp.

The cool state is characterized by sufficient strength and stiffness to permit a lens blank to be attached to a block, and by minimal apparent mass flow of the blocking composition under typical lens processing stresses and/or pressures at temperatures near or below room temperature.

The warm and cool state properties permit the blocking composition to be heated to a moderate temperature, shaped while warm to conform to the lens blank, and cooled or allowed to cool to form a substantially rigid block or blocking composition.

Suitable thermoplastic materials for use in the present invention include polyesters and polyurethanes such as those described in U.S. Pat. Nos. 3,382,202, 4,059,715, 4,182,829, 4,327,013, 4,361,538, 4,552,906 and 4,569,342; copolymers such as those described in U.S. Pat. Nos. 4,659,786 (e.g., polyester-polysiloxane block copolymers), 4,740,245 (e.g., ethylene vinyl acetate copolymers), and 4,768,951 (e.g., ionomer resins of ethylene copolymers); segmented copolymers and polyetheresters such as those described in U.S. Pat. Nos. 3,651,014, 4,173,506, 4,059,715, 4,066,600, 4,025,694, 4,430,429 and 4,552,906; ethylene vinyl acetate resins such as are described in European Published Pat. Application No. 0 359 135 and Kokai No. Sho 63[1988]-96536; blends of aromatic hydrocarbon resins and side chain crystallizable hydrocarbon polymers or copolymers; and polycaprolactones such as those described in U.S. Pat. Nos. 5,066,231, 5,040,976, and 5,026,278. The disclosures of these references are herein incorporated by reference for their teachings and disclosures of suitable thermoplastic materials.

Suitable thermoplastic materials have a weight average molecular weight of at least about 1,000. Preferred thermoplastic materials have a weight average molecular weight of between about 1,000 and 100,000; more preferred materials have a weight average molecular weight of between about 10,000 and 70,000; and most preferred materials have a weight average molecular weight of between about 12,000 and 65,000. Preferred thermoplastic materials have a number average molecular weight of between about 1,000 and 100,000; more preferred materials have a number average molecular weight of between about 3,000 and 50,000; and most preferred materials have a number average molecular weight of between about 4,000 and 45,000. Preferred ther-

moplastics materials have a polydispersity less than about 10; more preferred materials have a polydispersity less than about 8; and most preferred materials have a polydispersity less than about 6.

In one presently preferred embodiment, the thermoplastic material is a homopolymer or copolymer of epsilon-caprolactone. Preferred polycaprolactones have the general formula:



wherein  $R^1$  is an aromatic or a straight chain or branched aliphatic backbone, which can optionally contain one or more non-interfering substituents such as hydroxyl or amine groups,  $w$  is 1 if  $R^1$  is hydrogen, and  $w$  otherwise has an average value of about 1 to about 4,  $M$  is oxygen or  $-NR^2-$  where  $R^2$  is hydrogen or a non-interfering aromatic or aliphatic group, and the average product of  $w$  times  $x$  is preferably greater than about 35.

Blends of polycaprolactones can also be employed. Compositions containing a blend of high and low molecular weight polycaprolactones can have both a higher modulus and a lower viscosity than a composition containing only one of the constituent polycaprolactones. In other words, the blend provides a synergistic combination of modulus and low viscosity. For example, blends of high molecular weight polycaprolactones (e.g., with a number average molecular weight greater than about 20,000) and low molecular weight polycaprolactones (e.g., with a number average molecular weight less than about 20,000) may be used. If desired, more than one high or low molecular weight polycaprolactone may be used. For example, one may employ two different low molecular weight polycaprolactones and one high molecular weight polycaprolactone.

As used in this specification a "high molecular weight polycaprolactone" refers to an epsilon-caprolactone homopolymer or copolymer whose number average molecular weight is at least about 20,000, and preferably at least about 30,000. The high molecular weight polycaprolactones preferably have the general formula described above, wherein  $R^1$ ,  $R^2$ ,  $w$ , and  $M$  are as previously defined and the product of  $w$  times  $x$  is greater than about 175. The product of  $w$  times  $x$  is more preferably at least about 250 and most preferably between about 250 and 440.

The low molecular weight polycaprolactone is an epsilon-caprolactone homopolymer or copolymer whose number average molecular weight is less than about 20,000, and preferably less than about 10,000. The low molecular weight polycaprolactones preferably have the general formula described above, wherein  $R^1$ ,  $R^2$ ,  $w$ , and  $M$  are as previously defined and the product of  $w$  times  $x$  is less than about 175. The product of  $w$  times  $x$  is more preferably less than about 100, and most preferably between about 3 and 90.

As a further guide, when the composition comprises a blend of high and low molecular weight polycaprolactones, the weight ratio of high to low molecular weight polycaprolactones preferably is between about 9.5:0.5 to 0.5:9.5, more preferably between about 9:1 to 1:9, most preferably 50:50 to 1.5:8.5, and will depend in part on the intended use for the composition.

The polycaprolactone can contain property-modifying or cross-linkable functional groups (for example, hydroxyl, acrylate, methacrylate, epoxy, isocyanato, or vinyl groups) if desired.

Preferred commercially available high molecular weight polycaprolactone polymers include "TONE P-767" polycaprolactone from Union Carbide Corp., the "CAPA" polycaprolactones "640" (reported 40,000 molecular weight), "650" (reported 50,000 molecular weight) and "656" (reported 56,000 molecular weight) from Solvay Interox, and the various high molecular weight polycaprolactones available from Daicell Chemical Industry Co., Ltd. Other suitable high molecular weight polycaprolactone polymers include CAPA 630 from Solvay Interox.

Preferred commercially available low molecular weight polycaprolactone polymers include "TONE P-300" polycaprolactone (reported 10,000 molecular weight), "TONE 1270" polycaprolactone (reported 4,000 molecular weight), the "TONE" polycaprolactone diols "0200" (reported 530 molecular weight), "0210" (reported 830 molecular weight), "0230" (reported 1,250 molecular weight), "0240" and "2240" (reported 2,000 molecular weight), and "0250" (reported 3,000 molecular weight), "TONE" polycaprolactone triols "0301" (reported 300 molecular weight), "0305" (reported 540 molecular weight) and "0310" (reported 900 molecular weight) from Union Carbide Corp., as well as the "CAPA" polycaprolactone diols "203" (reported 400 molecular weight) through "240" (reported 4,000 molecular weight), "CAPA" polycaprolactone triols "304" (250 molecular weight) and "305" (reported 540 molecular weight), and the "CAPA" polycaprolactone tetraol "316" (reported 1,000 molecular weight) available from Solvay Interox.

The amounts of high molecular weight and/or low molecular weight polycaprolactone, and the amounts of other ingredients in the blocking compositions of the invention, usually will be empirically selected. Selection should be based in part on the desired end use for the composition and the desired properties in the molten or softened ("warm") and solid or hard ("cool") states. For polycaprolactones, the warm state is characterized by an amorphous microstructure, and by appreciable mass flow under moderate pressure at some temperature between about 35° C. and about 85° C., although a maximum of about 75° C. is preferred. The cool state is characterized by a solidified semi-crystalline polycaprolactone microstructure, and by minimal, preferably no, apparent mass flow under moderate pressure at temperatures below 21° C.

Blends of polycaprolactones with other suitable and compatible materials and polymers can also be employed. For example, a suitable polycaprolactone material may be blended with an ethylene vinyl acetate ("EVA") resin. Suitable EVA resins are described in European Published Pat. Application No. 0 359 135 and Kokai No. Sho 63[1988]-96536. Suitable commercially available EVA resins include the "ELVAX" resins shown below:

| ELVAX Resin | Melt flow rate | % Vinyl acetate |
|-------------|----------------|-----------------|
| 40-W        | 48-66          | 40              |
| 150         | 38-48          | 33              |
| 210         | 400            | 28              |
| 220         | 134-168        | 28              |
| 250         | 22-28          | 28              |
| 260         | 5.3-6.7        | 28              |
| 4969-6W     | 1900           | 28              |

These resins are commercially available from E. I. duPont de Nemours & Company. "ULTRATHENE" EVA resins from Quantum Chemical Corp. and "ESCORENE" EVA resins from Exxon Chemical Corp. are also useful. Blends of resins can be used if desired.

In another embodiment, the thermoplastic material comprises a blend of the aforementioned EVA resins with a suitable wax material (e.g., paraffinic hydrocarbons). Suitable wax materials include commercially available waxes such as "SHELLWAX" and "SHELLMAX" available from Shell Oil Company, Houston, Tex. and "EPOLENE" waxes available from Eastman Chemical Products, Inc. Kingsport, Tenn. "SHELLWAX" waxes are available in a variety of grades having melt points from 50° to 84° C. Suitable "SHELLWAX" waxes include grades 100, 120, 200, 270, 300, and 700. "SHELLWAX" grade 200 is presently particularly preferred. Suitable "EPOLENE" waxes are available in a variety of grades having molecular weights from about 1,800 to 23,000.

The preferred amounts of thermoplastic resin and wax in this embodiment of the thermoplastic blocking composition are as follows:

| Ingredient          | Preferred weight % | More preferred weight % |
|---------------------|--------------------|-------------------------|
| Thermoplastic resin | 30 to 90           | 50 to 80                |
| Wax                 | 10 to 70           | 20 to 50                |

In yet another embodiment, the thermoplastic material is a segmented copolyester, preferably consisting essentially of a multiplicity of recurring intralinear long chain and short chain ester units connected head-to-tail through ester linkages. These are solid, non-tacky, strongly cohesive, solvent-free thermoplastic polymers. They consist essentially of from about 5 to 75 percent by weight of amorphous ester units and 95 to 25 percent by weight of crystallizable ester units joined through the ester linkages (the term "crystallizable" as used herein includes both crystalline ester units and units which are capable of becoming crystalline).

The crystallizable ester units in the copolymers are of the formula:  $—C(O)R_1C(O)—OR_2O—$  (formula I) and the amorphous ester units are of the formula:  $—C(O)R_3C(O)—OR_4O—$  (formula II) wherein:

$R_1$  is preferably the divalent radical remaining after removal of carboxyl groups from a dicarboxylic acid having a molecular weight less than about 300, more preferably,  $R_1$  consists of residues (remaining after removal of the carboxyl groups) of one or more diacids selected from saturated aliphatic dicarboxylic acids containing from 4 to 10 carbon atoms (the residues thereof containing from 2 to 8 carbon atoms) and, alternatively and less preferably, aromatic dicarboxylic acids such as terephthalic acid, isophthalic acid, phthalic acid, 4-4'-benzophenone dicarboxylic acid, 4-4'-diphenylmethanedicarboxylic acid, 4-4'-diphenylether dicarboxylic acid, 4,4'-diphenylthioether dicarboxylic acid and 4,4'-diphenylamine dicarboxylic acid;

$R_2$  is preferably the divalent radical remaining after removal of hydroxyl groups from a low molecular weight diol having a molecular weight less than about 250, more preferably,  $R_2$  consists of residues (remaining after removal of the hydroxyl groups) of one or more saturated aliphatic diols containing from 2 to 12 carbon atoms;

$R_3$  is preferably  $R_1$ , optionally  $R_3$  is  $R_5$ , wherein  $R_5$  consists of the divalent radicals containing from 22 to 50 carbon atoms which remain after removal of the carboxyl groups from saturated aliphatic dimer acids (i.e., the polymerized and hydrogenated product of two molecules of an ethylenically unsaturated fatty acid

5  
10  
15  
20  
25  
30  
35  
40  
45  
50  
55

containing from about 12 to 26 carbon atoms, the dimer acid thus being saturated and containing from 24 to 52 carbon atoms); and

$R_4$  is  $R_2$  or  $R_6$ , wherein  $R_6$  consists of the divalent radicals remaining after removal of the hydroxyl groups from a long chain aliphatic diol having an average molecular weight of 200 to 4,000 (preferably 400 to 2,000, and more preferably 600 to 2,000), provided that at least one of  $R_3$  and  $R_4$  in each amorphous ester unit is  $R_5$  or  $R_6$ , and provided that when  $R_1$  is aromatic,  $R_2$  contains from 6 to 12 carbon atoms and the amorphous content is 50-75 percent by weight.

The copolymers preferably have DTA melting temperatures of from about 25° to 150° C. and inherent viscosities of preferably at least 0.5 dl/g (this and the other inherent viscosities herein are measured in 0.3 g/dl solutions of polymer in chloroform at 25° C.). Usually the inherent viscosities of the copolymers are not more than 1.5 dl/g at 25° C.

The copolymers of the present invention are preferably substantially linear and of relatively high strength. The linear copolymers are prepared from short and long chain precursors which are difunctional with respect to carboxyl and hydroxyl, for example organic diols (glycols) and dicarboxylic acids. The diacid precursors containing  $R_1$  are often 20 referred to herein as short chain diacids, the diol precursors containing  $R_2$  as short chain diols, the diacid precursors containing  $R_5$  as long chain diacids and the diol precursors containing  $R_6$  as long chain diols. The carboxyl and hydroxyl functions most often appear in the precursors as the free acid and free base but can also appear as simple derivative functions such as esters, acid chlorides or anhydrides if desired.

The relative amount of crystallizable and amorphous units is determined by the precursor charge. Most frequently the 25 copolymers are reaction products of a long and a short chain precursor of one functionality and a short chain precursor of the other functionality. In case of such a stoichiometrically balanced charge of three monomers, the weight percentages of amorphous and crystallizable units can be calculated 30 exactly (this is also true where there are more than three monomers but of only three types, e.g., two short chain diacids, one short chain diol and one long chain diacid but no long chain diol, etc.). However, if monomers of all four types are included in the charge, the relative amounts of 35 amorphous and crystallizable units are not exact but can be expressed as falling between two values (the range being quite narrow). Thus, to calculate the minimum amorphous 40 content in such a copolyester, it is assumed that the maximum possible reaction occurs between the short chain diol and short chain diacid (thus maximizing the content of 45 crystallizable units). To calculate the maximum amorphous content, it is assumed that the maximum possible reaction 50 occurs first between the short chain diacid and the long chain diol and between the short chain diol and the long chain diacid, the remaining reactants after those reactions (if any 55 remain) reacting with one another.

The amorphous and crystallizable units of the copolymers can alternate in the polymer chains or they can appear in blocks of the same type and this can be controlled to some extent by the process of preparation. For example, prepolymers of crystallizable and/or amorphous units can be prepared separately thus assuring larger blocks of one type or the other or, as is the usual practice, the precursors (monomers) can be charged directly and simultaneously to the reaction vessel.

The amorphous blocks of the copolymers of the invention are most often composed of alternating long chain diol

60  
65

and short chain diacid residues, but this is not necessarily the case. Although it is possible that a long chain diol and a long chain diacid could react alternately to form blocks of several repeating units, this is unlikely and, at any rate would have little effect on the properties of the resulting polymer. The end groups of the copolymers can be of a single functionality, if an excess of one precursor is included, or can be a mixture if the charge was stoichiometrically balanced.

The short chain diacids can be saturated aliphatic acids containing from 4 to 40 carbon atoms (including unbranched, branched, or cyclic having 5 to 6 atoms in a ring) and/or aromatic acids containing from 8 to 15 carbon atoms. Examples of suitable aliphatic acids are succinic, glutaric, adipic, pimelic, suberic, azelaic, sebacic, 1,3- or 1,4-cyclohexanedicarboxylic, 1,3-cyclopentanedicarboxylic, 2-methylsuccinic, 2-methylpentanedioic, 3-methylhexanedioic, carbonic, oxalic, itaconic, diethylmalonic, fumaric, citraconic, allylmalonate, 4-cyclohexene-1,2-dicarboxylate, 2,5-diethyladipic, 2-ethylsuberic, 2,2,3,3-tetramethylsuccinic, decahydro-1,5- (or 2,6-) naphthylene dicarboxylic, 4,4'-bicyclohexyl dicarboxylic, 4,4'-methylenebis(cyclohexyl carboxylic), 3,4-furan dicarboxylate, and 1,1-cyclobutane dicarboxylate acids and the like. Other representative dicarboxylic acids include terephthalic and isophthalic acids, bibenzoic acid, substituted dicarboxy compounds with benzene nuclei such as bis(p-carboxyphenyl) methane, p-oxy (p-carboxyphenyl) benzoic acid, ethylenebis(p-oxybenzoic acid), 1,5-naphthalene dicarboxylic acid, 2,6-naphthalene dicarboxylic acid, 2,7-naphthalene dicarboxylic acid, phenanthralene dicarboxylic acid, anthralene dicarboxylic acid, 4,4'-sulfonyl dibenzoic acid, etc. and C<sub>1</sub>-C<sub>10</sub> alkyl and other ring substitution derivatives thereof such as halo, alkoxy or aryl derivatives.

The short chain diols include branched, unbranched, and cyclic aliphatic diols having 2 to 15 carbon atoms, such as, for example, ethylene glycol, 1,3-propylene glycol, 1,2-propylene glycol, 1,4-butanediol, 1,3-butanediol, 1,5-pentanediol, 2-methyl-2,4-pentanediol, 1,6-hexanediol, 1,8-octanediol, cyclobutane-1,3-di(2'-ethanol), cyclohexane-1,4-dimethanol, 1,10-decanediol, and 1,12-dodecanediol. Preferred are diols with 2-15 carbon atoms such as ethylene, propylene, isobutylene, tetramethylene, pentamethylene, 2,2-dimethyltrimethylene, hexamethylene and decamethylene glycols, dihydroxy cyclohexane, cyclohexane dimethanol, resorcinol, hydroquinone, 1,5-dihydroxy naphthalene, etc. Especially preferred are aliphatic diols containing 2-8 carbon atoms. Included among the bis-phenols which can be used are bis(p-hydroxy) diphenyl, bis(p-hydroxyphenyl) methane, and bis(p-hydroxyphenyl) propane.

The chemical structure of the long chain diol is not critical. Any substituent groups which do not interfere with the polymerization reaction to form the copolyester can be present. Thus, the chain can be a single divalent acyclic or alicyclic, hydrocarbon group, poly(alkylene oxide) group, polyester group, a combination thereof, or the like. Any of these groups can contain substituents which do not interfere to any substantial extent with the polymerization to form the copolyester used in accordance with this invention. The hydroxy functional groups of the long chain diols used to prepare the copolymers should be terminal groups to the extent possible.

Suitable long chain diols include poly(oxyalkylene) glycols in which the alkylene group contains from 2 to 9 carbon atoms, preferably from 3 to 8 carbon atoms and more

preferably from 2 to 4 carbon atoms. Among these compounds are poly(alkylene oxide) glycols and polyether glycols such as poly(oxyethylene)glycols having molecular weights of about 200, 600, 1500, and 2000, poly(oxypropylene)glycols, having molecular weights of about 425 and 1800, poly(oxytetramethylene)glycols, poly(oxypentamethylene)glycol, poly(oxyhexamethylene)glycols, poly(oxyheptamethylene)glycols, poly(oxyoctamethylene)glycols, poly(oxynonamethylene)glycols, poly(1,2-butylene oxide)glycol, random or block copolymers thereof, for example, glycols derived from ethylene oxide and 1,2-propylene oxide and poly-formals prepared by reacting formaldehyde with glycols, such as pentamethylene glycol, or mixtures of glycols, such as a mixture of tetramethylene and pentamethylene glycols. Also included are poly(lactone)glycols, e.g., poly(caprolactone) glycol; poly(oxyalkylenecarbonate)glycols, e.g., poly(oxyethylenecarbonate)glycol; and glycols containing a hydrocarbon main chain, e.g., hydroxy-terminated polybutadiene.

The copolymers can be prepared by conventional polycondensation polyester-forming reactions wherein one or more short chain diacids and/or long chain diacids or their equivalents (e.g., volatile alcohol esters, acid chlorides, or anhydrides of the diacids) are caused to react with an equivalent amount of one or more short chain diols and/or long chain diols. When copolymers having an acid value of no more than about 2 (indicating substantially complete reaction) and relatively high molecular weight are desired, it is preferable that the polyester reaction be carried out in the presence of a suitable catalyst.

The choice of catalyst depends on the starting materials. Thus, for simple esterification of a short chain diacid with a short chain diol and a long chain diol, the diacid alone may preferably function as esterification catalyst. Optionally, however, one may use as a catalyst a compound having an ionization constant greater than about 10<sup>-3</sup>, such as, for example, p-t-butylbenzenesulfonic acid. For esterification by ester interchange, an ester interchange catalyst is used. Suitable catalysts include, for example, manganous acetate, calcium acetate, zinc acetate, sodium methoxide, antimony oxide, antimony glyoxide, tetraalkyltitanates, complex titanates such as magnesium hexaalkyltitanates or other suitable ester interchange catalysts as described in the literature relating to the preparation of polyesters.

In yet another embodiment, the thermoplastic material is a blend of (i) a hydrocarbon resin, preferably an aromatic hydrocarbon resin; (ii) a side chain crystallizable hydrocarbon polymer or copolymer; and optionally (iii) a modifier or mixture of modifiers, preferably straight chain alcohols.

A wide variety of hydrocarbons resins may be employed in these compositions. Aliphatic resins, aromatic resins, mixed aliphatic/aromatic resins, hydrogenated pure aromatic resins, and hydrogenated mixed aromatic resins may be used. Preferred hydrocarbon resins have Ring and Ball Softening Points from about 70° to 110° C., more preferably from about 80° to 100° C., and most preferably from about 86° to 90° C. Preferred weight average molecular weight of the hydrocarbon resin is from about 450 to 1650, more preferably from about 450 to 1,200, and most preferably from about 450 to 925. Suitable hydrocarbon resins include REGALITE R-91, PICCOTAC 95, PICCOLYTE HM90, REGALREZ 1085 and 1094, and KRISTALEX 3085 (available from Hercules, Inc.). Preferably, the blend of this embodiment comprises between 30 and 65 weight percent hydrocarbon resin, more preferably between 40 and 65 weight percent hydrocarbon resin, and most preferably between 50 and 65 weight percent hydrocarbon resin.

Suitable side chain crystallizable hydrocarbon polymers or copolymers for use in these compositions include polymers based on an ethylene structure having pendant hydrocarbon side chains. These polymers are sometimes termed "poly alpha olefins" or "poly 1-alkenes." Preferred side chain crystallizable hydrocarbon polymers or copolymers have an average of at least about eight carbons in the side chain. Preferred side chain crystallizable hydrocarbon polymers or copolymers have Ring and Ball Softening Points from about 54° to 75° C., and more preferably from about 10 65° to 75° C. Preferred number average molecular weight of the side chain crystallizable hydrocarbon polymer or copolymer is from about 500 to 3,000. Suitable side chain crystallizable hydrocarbon polymers include "VYBAR" 103 and 15 253 from Petrolite Corp. Blends of these polymers may be used if desired. Additionally, copolymers of ethylene with poly 1-alkenes are believed to be useful for this invention. Preferred 1-alkene comonomers have carbon length of at least about 10 carbons. Preferably, the blend of this embodiment comprises between 20 and 70 weight percent side 20 250 chain crystallizable hydrocarbon polymer or copolymer, more preferably between 25 and 60 weight percent side chain crystallizable hydrocarbon polymer or copolymer, and most preferably between 30 and 50 weight percent side 200 chain crystallizable hydrocarbon polymer or copolymer.

The blend of this embodiment may optionally comprise a modifier such as the viscosity modifiers and/or performance modifiers described below. Suitable modifiers for this blend include: carboxylic acids of the general form  $\text{CH}_3(\text{CH}_2)_n\text{COOH}$ , where n is between about 10 and 16; straight chain monohydric alcohols of the general form  $\text{CH}_3(\text{CH}_2)_n\text{OH}$ , where n is between about 11 and 19; and branched chain monohydric alcohols having between 10 and 20 carbon atoms. Polyethylene glycols and polyethylene glycol ether modifiers, which may be suitable for other embodiments of the invention, are not preferred for this embodiment. Suitable alcohols include straight chain alcohols and branched chain alcohols, with straight chain alcohols being preferred for these blends. Preferred modifiers for the blend comprise straight chain alcohols having the general formula  $\text{CH}_3(\text{CH}_2)_n\text{OH}$ , where n is preferably between about 11 and 19 for blocking compositions that have a melting temperature between about 45° and 75° C. More preferably, n is between about 13 and 17 for these compositions. In general, the number of  $-\text{CH}_2-$  groups may be adjusted to complement the particular thermoplastic blocking composition blend being used. Higher numbers of these groups tend to increase the melting temperature of the alcohol. Thus, when the melting temperature of the blocking composition blend being used is higher than 75° C., the number of  $-\text{CH}_2-$  groups can be larger. Conversely, alcohols having lower numbers of  $-\text{CH}_2-$  groups will tend to be liquids at room temperature. Their use in a blocking composition may result in a blend that has a somewhat greasy feel. Particularly preferred monohydric straight chain alcohol modifiers for use with blends of hydrocarbon resins and side chain crystallizable hydrocarbon polymers or copolymers include 1-octadecanol ("stearyl alcohol," available from Aldrich Chem. Co., Milwaukee, Wis.), 1-hexadecanol ("cetyl alcohol," available from Aldrich Chem. Co.), 1-tetradecanol ("myristyl alcohol," available from Aldrich Chem. Co.), and 1-dodecanol ("dodecyl alcohol," available from Eastman Chem. Products, Inc., Kingsport, Tenn.). Stearyl alcohol and myristyl alcohol are particularly preferred for these blends. Blends of both these alcohols are especially preferred.

Suitable blends comprise up to about 15 weight percent alcohol modifier. The blend of this embodiment preferably

comprises between 0.5 and 15 weight percent modifier, more preferably between 2 and 10 weight percent modifier, and most preferably between 3 and 8 weight percent modifier. The blend of this embodiment may also comprise a suitable amount of an antioxidant. For example, approximately 1 weight percent BHT has been found to be suitable.

Suitable thermoplastic materials have a melting or softening point above about 35° C. Preferred thermoplastic materials have a melting or softening point between about 40° and 85° C., more preferably between about 45° and 75° C., and most preferably between about 50° and 70° C. A composition has reached its melting or softening point when it has changed from its solid state and has become capable of appreciable mass flow under moderate pressure.

Preferred compositions are capable of being injection molded using standard blocking apparatus. Typically, the pressure employed in commercial blocking apparatuses is about 69 kPa (10 psi). Preferred compositions for forming blocks are able to fill the lens block cavity in less than about 2 minutes using standard equipment, such as an "OPTEK" 200 blocker from Optek Division, Associated Development Corp., Pinellas Park, Fla. More preferably, the cavity can be filled in less than about 1 minute, and most preferably, the cavity can be filled in less than about 30 seconds.

A common physical property measured in the plastics 25 industry to characterize a material's flow properties under pressure is its viscosity. Suitable compositions have a viscosity that is low enough such that the material may be easily molded when in its warm state to the shape of the lens blank. Preferred materials have a viscosity that is low 30 enough such that the material may be injection molded within a reasonable time under a reasonable pressure. The composition's viscosity is preferably not so low that the composition undesirably "flashes" when injection molded (i.e., undesirably flows through cracks between the cavity 35 and the lens blank). In addition, when the composition contains solid adjuvents, such as fillers, the warm state viscosity should preferably be high enough that the filler does not undesirably settle.

Preferred blocking compositions for use in the present 40 invention with traditional blocking machines have a shear viscosity (measured at the desired temperature of use using a Rheometrics Dynamic Analyzer (RDA-II) having 25 mm parallel plate geometry and a steady shear rate of  $1 \text{ s}^{-1}$ ) of between 3 and 500 Pascal seconds (Pa s). More preferred 45 blocking compositions for use in the present invention with traditional blocking machines have a shear viscosity of between 3 and 100 Pa s. Most preferred blocking compositions for use in the present invention with traditional blocking machines have a shear viscosity of between 3 and 50 Pa s.

The blocking composition should preferably be hard 55 enough at its use temperature to function in the manner intended. For example, the composition, when used to form a complete block, should be hard enough to withstand the forces and stresses imparted during the typical lens processing procedure, including any forces and stresses imparted to the composition during mounting and unmounting from the lens processing machinery as well as any forces imparted to the composition during the actual grinding or finishing 60 operation. Compositions that deform or flow appreciably during these operations may be unsuitable. Suitable thermoplastic materials are solid or "hard" at temperatures near or below room temperature. Preferred thermoplastic materials are solid at temperatures below about 40° C., more preferred thermoplastic materials are solid at temperatures below about 45° C., and most preferred thermoplastic materials are solid at temperatures below about 50° C.

**15**

The hardness of the blocking composition may be measured by the material's bending modulus. This property is conveniently measured using the three-point bending technique described in ASTM D790-86. Suitable blocking compositions have a mean bending modulus of at least 34.4 MPa, preferably at least 69 MPa, more preferably at least 138 MPa, and most preferably at least 276 MPa, when tested at 21° C. according to ASTM D790-86 (using at least 3 specimens per test).

Preferred solid blocking compositions exhibit a Shore "A" hardness of at least 40 when tested at 21° C. using the technique described in ASTM D2240 (using at least 3 specimens per test). More preferred compositions have a Shore "A" hardness of at least 70, and most preferred compositions have a Shore "A" hardness of at least 90. If the Shore "A" value of a particular material is out of scale then Shore "D" may be employed. More preferred solid blocking compositions exhibit a Shore "D" hardness of at least 20 when tested at 21° C. using the technique described in ASTM D2240 (using at least 3 specimens per test). Most preferred compositions have a Shore "D" hardness of at least 25, and optimum compositions have a Shore "D" hardness of at least 30.

Alternatively, the hardness of the composition may be tested using a nanoindentation technique, as described in Example 2. Preferred compositions have a nanoindentation hardness of at least 1 GPa, more preferred compositions have a nanoindentation hardness of at least 2 GPa, and most preferred compositions have a nanoindentation hardness of at least 4.5 GPa.

The blocking composition should preferably have enough cohesive strength and/or tensile strength to function in the manner intended. For example, the composition, when used to form a complete block, should have enough cohesive strength to withstand the forces and stresses imparted during the typical lens processing procedure, including any forces and stresses imparted to the composition during mounting and unmounting from the lens processing machinery as well as any forces imparted to the composition during the actual grinding or finishing operation. Compositions that fall apart, crack, or shatter during these operations are unsuitable.

The strength of the blocking composition may be conveniently measured using the three-point bending technique described in ASTM D790-86. Preferred blocking compositions have a mean flexural strength at 21° C. of at least 1 MPa, more preferably at least 2 MPa, most preferably at least 4 MPa, and optimally at least 6.8 MPa, when tested according to ASTM D790-86 (using at least 4 specimens per test).

The blocking composition preferably should be dimensionally stable and should maintain the desired geometric alignment of the lens blank to the processing machine. Compositions that are either too soft or that creep under typical operating stresses may not maintain the necessary alignment of the lens to the reference guides on the back of the block. These errors will be imparted to the lens and may cause imprecise machining of the lens.

Preferred blocking compositions are relatively dimensionally stable when heated over a temperature range of 0° C. to near the melting temperature of the composition. Example 1 describes a Thermal Mechanical Analysis technique that may be used to measure a material's dimensional change upon heating. Preferred blocking compositions exhibit less than 2.9% change in dimension over a temperature range between 0° C. and three degrees less than the material's melting temperature, when tested according to the procedure described in Example 1. More preferred blocking

**16**

compositions exhibit less than 2% change in dimension, and most preferred blocking compositions exhibit less than 1.5% change in dimension.

Preferred blocking compositions are also relatively dimensionally stable when cooled over a temperature range of near the melting temperature of the composition to 21° C. Preferred blocking compositions exhibit less than a 5% change in volume when cooled from the material's melting temperature to 21° C. More preferred blocking compositions exhibit less than 4% change in volume, and most preferred blocking compositions exhibit less than 3% change in volume. Optimally, the blocking composition can withstand normal changes in dimension without cracking or crazing.

The blocking composition is preferably non-tacky at 21° C. Materials which are tacky at room temperature tend to be difficult to work with and messy. Tacky materials also tend to become contaminated with lint and dust. These contaminants can adversely affect the ability of the composition to be recycled. Tackiness may be measured using a probe tack test as described in ASTM D2979-88 and Example 2 below. Preferred compositions have a mean peak value of less than 800 g, more preferred compositions have a mean peak value of less than 400 g, when tested as described herein.

The blocking composition should preferably adhere to the lens blank (or to a coating or tape applied to the lens blank) with a sufficient strength to avoid unintended detachment of the lens during processing, yet preferably allow deblocking of the lens using traditional shock deblocking or hot-water deblocking methods. Thus, a preferred balance of adhesion should be achieved.

One method of measuring adhesion is described in Example 2. This method utilizes a tensile testing machine to shear a small button of material from the surface of a substrate. Using this method, preferred blocking compositions have a mean shear adhesion value, of at least 6.5 kg/cm<sup>2</sup>, more preferably between 6.5 and 25 kg/cm<sup>2</sup>, and most preferably between about 8 and 20 kg/cm<sup>2</sup>.

Another method of assessing whether a particular blocking composition achieves the necessary balance of adhesion between the blocking composition and the lens blank (or to a coating or tape applied to the lens blank) is to perform a shock deblocking test using a standard commercial lens block. For this test, a 70 mm plastic lens with a 2.0–2.4 mm center thickness, piano, finished uncut, "RLX Plus™ Scratch Resistant, Finished Lens in Hard Resin" from Signet Armorlite, Inc. is optionally covered with a surface protective tape. A brass blocking ring is placed on a blocker (e.g., OPTEK™ Model 200 Blocker) and a 56 mm diameter Coburn Block from Coburn Company is placed into the ring such that the inlet in the block fits snugly over the rubber nozzle. The block is then centered on the lens and slowly filled with molten blocking composition. The blocked lens assembly is allowed to set for 10 to 15 seconds after filling, in order for the resin to harden and form a good bond to the taped lens. The blocked lens is removed from the blocker and allowed to set for 1 hour before deblocking. The blocked lens is placed into the deblocking ring and the lens is taped to the deblocking ring using 1.27 cm wide filament tape. With the blocking tool facing downward, the blocked lens is placed in a hollow tube. The diameter of the tube is much greater than the blocking tool and the tube is sufficiently thick to abruptly stop the lens by its perimeter. The blocked lens assembly is dropped starting at 2.54 cm height and raised in 2.54 cm increments until the block separated from the tape or until 15.24 cm in height, then, raised and dropped in 5.08 cm increments up to 91.44 cm. The height in centimeters at which the block released from the tape is

recorded as the deblock value. Using this method, preferred blocking compositions have a deblock value of between 5 and 56 cm, more preferably between 7 and 45 cm, most preferably between about 10 and 35 cm, and optimally between about 14 and 20 cm.

The blocking compositions of the present invention can contain a wide variety of adjuvants depending upon the desired end use. Suitable adjuvants include solvents, diluents, plasticizers, pigments, dyes, inorganic and organic fibrous or particulate reinforcing or extending fillers, nucleating agents, thixotropic agents, indicators, inhibitors, stabilizers, UV or IR absorbers, and the like.

Viscosity modifiers and/or performance modifiers (hereinafter "modifiers") are particularly preferred optional adjuvants for use with the thermoplastic blocking compositions of the present invention. These modifiers may be added to the blocking composition as needed to either enhance or adjust certain warm state properties, such as the viscosity of the heated composition (e.g., to facilitate flow rates during cavity filling) and/or to enhance or adjust certain cool state properties, such as resistance of the material to cracking upon cooling. Preferably, the modifiers are essentially solid at room temperature (so as to not undesirably provide a "greasy" feel to the blocking composition). The modifiers also preferably maintain their compatibility with the blocking composition during their transition to or from the cool state to the warm state. Most preferably, the modifier does not undesirably phase separate during these transitions.

Suitable modifiers include carboxylic acids of the form  $\text{CH}_3(\text{CH}_2)_n\text{COOH}$ , where n is preferably between about 10 and 16 for blocking compositions that have a melting temperature between about 45° and 75° C. In general, the number of  $-\text{CH}_2-$  groups may be adjusted to complement the particular thermoplastic blocking composition being used. Higher numbers of these groups tend to increase the melting temperature of the acid. Thus, when the melting temperature of the blocking composition being used is higher than 75° C., the number of  $-\text{CH}_2-$  groups can be larger. Conversely, acids having lower numbers of  $-\text{CH}_2-$  groups will tend to be liquids at room temperature. Their use in a blocking composition may result in a blend that has a somewhat greasy feel. A particularly preferred carboxylic acid modifier for use with polycaprolactone polymers and blends of polycaprolactone polymers is 1-octadecanoic acid ("stearic acid," available from Aldrich Chem. Co., Milwaukee, Wis.).

Suitable blocking compositions have been developed that incorporate between about 0 and 40 weight percent carboxylic acid modifier. More preferably, polycaprolactone based blocking composition comprise between about 1 and 25 weight percent carboxylic acid modifier, and most preferably, between about 5 and 20 percent carboxylic acid modifier.

Other suitable modifiers include monohydric and polyhydric alcohols. Suitable alcohols include straight chain alcohols, branched chain alcohols and glycols. Preferred monohydric straight chain alcohols have the general form  $\text{CH}_3(\text{CH}_2)_n\text{OH}$ , where n is preferably between about 11 and 19 for blocking compositions that have a melting temperature between about 45° and 75° C. More preferably, n is between about 13 and 17 for these compositions. In general, the number of  $-\text{CH}_2-$  groups may be adjusted to complement the particular thermoplastic blocking composition being used. Higher numbers of these groups tend to increase the melting temperature of the alcohol. Thus, when the melting temperature of the blocking composition being used is higher than 75° C., the number of  $-\text{CH}_2-$  groups can be

larger. Conversely, alcohols having lower numbers of  $-\text{CH}_2-$  groups will tend to be liquids at room temperature. Their use in a blocking composition may result in a blend that has a somewhat greasy feel. In general, suitable branched chain alcohols may have a somewhat larger number of  $-\text{CH}_2-$  groups than straight chain alcohols. Preferred branched chain alcohols have between 10 and 20 carbon atoms.

Particularly preferred monohydric straight chain alcohol modifiers for use with polycaprolactones and blends of polycaprolactones include 1-octadecanol ("stearyl alcohol," available from Aldrich Chem. Co., Milwaukee, Wis.), 1-hexadecanol ("cetyl alcohol," available from Aldrich Chem. Co.), 1-tetradecanol ("myristyl alcohol," available from Aldrich Chem. Co.), and 1-dodecanol ("dodecyl alcohol," available from Eastman Chem. Products, Inc., Kingsport, Tenn.).

Suitable blocking compositions comprise up to about 60 weight percent alcohol modifier. Preferred compositions comprise between about 1 and 60 weight percent alcohol modifier. More preferably, polycaprolactone based blocking compositions comprise between about 5 and 45 weight percent alcohol modifier, and most preferably, between about 15 and 40 percent alcohol modifier.

Preferred polyhydric alcohols include polyethylene glycols having the general form  $\text{H}(\text{OCH}_2\text{CH}_2)_n\text{OH}$ , where n is between 20 and 185, and polyethylene glycol ethers having the general form  $\text{R}(\text{OCH}_2\text{CH}_2)_n\text{OR}$ , where R is typically hydrogen or a straight-chain or branch-chain alkyl group having between 1 and 10 carbon atoms and where n is between 17 and 116. More preferably, one R group is hydrogen and the other R group is selected from the group consisting of  $\text{CH}_3$  and  $\text{CH}_2\text{CH}_3$ .

Most preferably, the polyhydric alcohol is a polyethylene glycol. Preferred polyethylene glycols have a weight average molecular weight between about 900 and 8,000. More preferably, for use with polycaprolactone based blocking compositions the polyethylene glycol has a weight average molecular weight between about 1,000 and 3,400. A presently preferred polyethylene glycol is available from Aldrich Chemical Company, Milwaukee, Wis., and has a molecular weight of about 1,500.

Other suitable polyhydric alcohols include polyethylene glycol methyl ethers having a weight average molecular weight between about 750 and 5,000. More preferably, for use with polycaprolactone based blocking compositions the polyethylene glycol methyl ether has a weight average molecular weight between about 1,000 and 3,400. A presently preferred polyethylene glycol methyl ether is available from Aldrich Chemical Company, Milwaukee, Wis., and has a molecular weight of about 2,000.

If desired, blends of two or more modifiers may be employed. For example, combinations of stearic acid and stearyl alcohol; stearyl alcohol and myristyl alcohol; stearyl alcohol, myristyl alcohol and dodecyl alcohol; and stearyl alcohol, myristyl alcohol and polyethylene glycol have been found to be beneficial. Other combinations will likely also be suitable. The blend should be chosen to optimize the properties of the blocking composition for its desired use. Myristyl alcohol has been found to be particularly compatible with polycaprolactone based blocking compositions and has also been found to help make other less compatible modifiers compatible with polycaprolactone. When blends of two or more modifiers are employed, suitable blocking compositions comprise up to about 60 weight percent of the blend of modifiers. Preferably, polycaprolactone based blocking compositions comprise between about 1 and 60

weight percent of the blend of modifiers, more preferably between about 15 and 50 weight percent of the blend of modifiers, and most preferably, between about 15 and 40 percent of the blend of modifiers.

Preferred fillers for use in the present invention comprise inorganic or organic, particulate or fibrous materials which are substantially insoluble in the continuous phase. Filler morphologies may include spheres, bubbles, expandable bubbles, particulate materials, filaments, microfibers, flakes and platelet type materials, as well as combinations of these. The fillers may have a solid, porous, or hollow structure.

Suitable inorganic filler materials include glass, amorphous and crystalline silica, soda lime borosilicate, amorphous sodium/potassium/aluminum silicate glass, alumina, iron oxides, calcium metasilicate, calcium carbonate, calcium sulfate (in either a particulate or microfiber form), kaolin, mica, talc, barium sulfate, boron fibers, carbon fibers, glass fibers, ground glass fibers, flake glass, metallic fibers, feldspar, barium ferrite, titanium oxide, ceramics and the like. Preferred inorganic filler materials include glass and ceramic bubbles such as: Scotchlite™ brand glass bubbles H50/10000 EPX, H50/10000 (acid washed), K-46, and S60/10000 (available from 3M); Extendosphere™ brand SG, CG, SF-12 (available from PQ Corp.); Zeeosphere™ brand 200, 400, 600, 800, and 850 (available from 3M); Zeolite™ W1000, W1012, W1300, W1600, G3400, and G3500 (available from 3M); Dicaperl™ brand HP-900 and HP-920 (available from Grefco) and Sil-Cell™ brand Sil-35/34, Sil-32, Sil-42, and Sil-43 (available from Silbriko Corp., Hodgkins, Ill. 60525). Dicaperl™ brand HP-820, HP-720, HP-520, HP-220, HP-120, HP-900, HP-920, CS-10-400, CS-10-200, CS-10-125, CSM-10-300, and CSM-10-150 (available from Grefco, Torrance, Calif.), and ceramic particles such as Cerameel™ (available from Microcel Tech. Inc.) may also be suitable, particularly when blended with other fillers. Colored pigment fillers are also suitable. Blends of these fillers may also be suitable.

Suitable organic fillers include fillers comprised of thermoplastic or thermoset organic materials or both as well as composite filler materials comprising the aforementioned organic materials as matrix and inorganic micro-inclusions dispersed therein. Preferred organic fillers are insoluble in the blocking composition. Suitable thermoplastic filler materials include polyolefins such as Primax brand UH-1080, UH-1060 and UH-1250 (available from Air Products & Chemicals—Allentown, Pa.), polyesters (e.g., poly(ethylene terephthalate), hereinafter referred to as “PET”), polyamides, polyimides, polyacrylates, polycarbonate, polyurethane and the like including copolymers of the aforementioned materials. Suitable thermoplastic filler materials also include expandable bubbles such as Expance 461 DE 20 microspheres (available from Nobel Industries). Suitable thermoset filler materials include epoxies, aldehyde condensation products (e.g., Ucar Thermoset microballoons BJO-0950, BJO-0820, BJO-0900, BJO-0840, BJO-09300 available from Union Carbide, Danbury, Conn.), acrylates, and methacrylates. Preferred organic filler materials include polyethylene microspheres (available from Air Products & Chemicals—Allentown, Pa.).

Preferred particulate fillers have an average particle diameter between 5 and 500 microns, more preferably the particulate fillers have an average particle diameter between 20 and 200 microns, most preferably the particulate fillers have an average particle diameter between 30 and 120 microns. As used herein, “average particle diameter” is defined as the diameter of a sphere of the same volume as the particle.

Microfibers may be added to the blocking composition to enhance integrity or composite strength. Preferred fibers for

use in the present invention have an average length between 25 and 5,000 microns, more preferably the fibers have an average length between 30 and 1,000 microns, most preferably the fibers have an average length between 30 and 500 microns. Microfiber fillers such as those described in U.S. patent application Ser. No. 08/008,751, which is herein incorporated by reference, may also be useful alone or in combination with other particulate fillers or fibers.

Suitable concentrations of filler in the blocking composition (i.e., “filler loading”) will vary depending on the bulk density of the filler, the specific gravity of the filler and particular thermoplastic blocking composition employed, and the desired handling property of the composition. A suitable filler loading is determined by selecting a level which is sufficiently high to ensure adequate strength but not so high that the composition becomes too viscous to flow and adapt to the lens surface when softened.

The composition should remain substantially homogeneous (that is, it should not undergo macroscopic phase separation or filler sedimentation) during use and more preferably during prolonged storage prior to use. The composition preferably should retain its desired physical properties even if repeatedly cycled between the warm and cool states. Thus the selection of ingredients can be guided in part by a desire to preserve homogeneity and thermal reversibility.

The ingredients in the blocking composition can be blended by hand or by mechanical mixing. The ingredients preferably are warmed sufficiently to melt the thermoplastic material, but if desired can be mixed at lower temperatures. Any suitable mixing device can be used, including kettles equipped with a mechanical stirrer, extruders, rubber mills, and the like.

The blocking composition can be put up in a variety of forms including preformed blocks, sheets, ropes, pellets, powders and the like. The composition can be shaped in a variety of ways including extrusion, injection molding and web processing using a coating knife or rollers. The composition can be sold unwrapped, loosely wrapped in a package, or packaged in tubes, syringes, and the like.

The blocking composition can be converted from the cool state to the warm state by using a variety of energy sources. The composition can be immersed in a heated bath containing a suitable inert liquid (e.g., water or a fluorochemical fluid) that will not dissolve or swell the composition in either its cool or warm states. The composition can also be softened using heat sources such as a melting pot, hot air gun, hot plate, conventional oven, infrared heater, or microwave oven. The composition can be encased in a plastic pouch, syringe or other container which is in turn heated or is subjected to one or more of the above-mentioned heating methods.

Transforming the blocking composition from a warm state to a cool state requires loss of thermal energy and can be carried out using a variety of cooling techniques. Cooling can take place under ambient conditions in the presence of air only. Cooling can also be expedited using forced air, cold water, ice, or heat sinks such as chilled “cold pack.” In one presently preferred method, the blocking composition is cooled using “cooling” or “chill” rings. The rings are shaped to surround the block and circulate a cool liquid, such as chilled water, thus dissipating heat from the blocking composition.

In one embodiment of the present invention, a composition, preferably comprising a “heat absorbing material,” is preformed into a “stock” lens block (e.g., by injection molding techniques). The generally concave sur-

face of the stock lens block is then heated, for example, using an infrared (IR) heat source, to melt the surface of the preformed block to a depth sufficient to allow the preformed block to conform to the surface of the lens blank. A lens blank is then positioned against the softened surface of the block and the heated surface is allowed to cool. Alternatively, the composition containing the heat absorbing material may be provided in a powdered, pelleted or sheet form and placed in the cavity of a block. The composition may then be heated as described above.

This method has the advantage that less material needs to be heated. Consequently, the procedure is very fast (sufficient surface heating can occur in less than about 10–15 seconds). In addition, the material is not stored in its warm state for a prolonged period (such as would occur in a melting pot). Thus, compositions having less long-term stability in the warm state may be employed.

Suitable “heat absorbing materials” include carbon black, and other inorganic pigments and fillers. The heat absorbing materials are preferably present in an amount sufficient to speed the heating of the blocking composition. Preferred compositions contain up to about 70% by weight of a heat absorbing material. More preferred compositions contain between about 1 and 20% by weight of a heat absorbing material, most preferred compositions contain between about 5 and 15% by weight of a heat absorbing material. The amount of the heat absorbing material may be empirically selected to adjust the depth of the softening layer for a given intensity IR source and a given exposure time.

If desired, a preformed stock lens block base can be fitted with a layer of a blocking composition of the present invention. Preferably, the layer comprises a heat absorbing material as described above. Desirably, the layer of blocking composition is thick enough to allow the heated layer to “conform” to the surface of the lens blank.

The blocking composition of the present invention is preferably utilized in conjunction with a suitable lens blank coating or tape. Preferred tapes for use with the blocking composition have a pressure-sensitive adhesive surface and a tack-free adhesion promoting surface. The tapes assist in the firm bonding of the lens blank to the lens block (i.e., the pressure sensitive adhesive on the tape firmly bonds to the lens blank and the thermoplastic lens blocking composition firmly adheres to the tack-free backside of the tape when applied thereto in the warm state and cooled). In addition, preferred tapes are conformable, that is, they follow the curvature of the lens blanks without any wrinkles or air bubbles; and translucent, that is, they permit light to pass therethrough. As a result, the lens may be visually aligned in the appropriate device prior to blocking. Still further, when preferred tapes of the present invention are removed from the lens they leave virtually no adhesive residue. Thus, messy and time consuming cleaning operations need not be performed on the lens before it can be used.

Despite this clean removability, suitable tapes of the present invention exhibit excellent adhesion to both the lens blank and the thermoplastic blocking composition. Additionally, the tapes of the invention are able to withstand the shear forces encountered during the surfacing and edging operations. As a result, lenses are held in accurate position throughout these operations. An added benefit offered by the tape of the present invention is the protection provided to the lenses from thermal and mechanical shock.

The composition of the exposed surface of the tape (i.e., the non-adhesive surface away from the lens blank) should be selected so as to achieve the desired degree of adhesion with the particular thermoplastic blocking composition. The

blocking compositions described herein generally comprise varying amounts of polar constituents or groups. While not intending to be bound by theory, it is presently believed that the polar constituents or groups present in certain blocking compositions of the present invention may interact with the polar groups present in certain tape backings and thus contribute to the adhesion between the tape surface and the thermoplastic composition (e.g., through a hydrogen bonding mechanism). According to this theory, the amount of available polar constituents or groups in both the blocking composition and at the surface of the tape would impact the total amount of adhesion between the composition and the tape.

The tapes are easily applied to ophthalmic lens blanks. Generally, the pressure-sensitive adhesive portion of the are applied to the front, or finished, surface of a lens blank. This may be done either by hand or, preferably, by means of a mechanical device. In either event, the tape conforms readily to the configuration of the lens blank without wrinkles, folds, air bubbles, or other discontinuities between the adhesive and the front surface of the lens. Preferably, the tape is applied so that it covers the entire front surface or back surface of the lens. Normally it is applied to the front surface.

The tapes may be used on both plastic and glass lens blanks which may vary in curvature from plano to 10-base curve or higher. It is, of course, understood that the particular tape employed may be selected to suit the particular lens to be altered. Preferably, more conformable tapes are employed with lens blanks having a higher base curvature.

After application, excess tape is trimmed away from the periphery of the lens blank. The lens blank is then blocked. After the blocking composition has solidified and cooled, the blocked lens is removed from the blocking machine and is ready for mounting in the surfacing and/or edging machines. When these operations have been completed, the finished lens is deblocked, for example, by means of a sharp tap. This may be easily accomplished, for example, with the aid of a hollow cylinder that is adapted to support the finished lens on its wall while receiving the still attached lens blank within its hollow portion. By holding the lens and cylinder together and striking the bottom of the cylinder upon a hard surface, the bond between the blocking composition and the tape may be broken. The lenses may also be deblocked, for example, by melting the blocking composition in hot water. In either event, the tape is then removed from the lens and discarded. The lens and block may then, if necessary, be cleaned.

The blocking composition of the present invention is preferably utilized in conjunction with a suitable preformed base block. Preferred base blocks are designed so that the blocking composition and base block form a unitary structure that securely holds the lens during processing. More preferably, the base block and composition are easily separated after use so that the base block and/or the composition may be reused or recycled.

A presently preferred base block contains a rear portion that is sized and adapted to fit the chuck of a desired lens processing machine and a front portion that is adapted to retain a blocking composition. The exact size and shape of the rear portion of the preformed base block may assume a variety of configurations. The preferred preformed base block also has a “negatively” tapered peripheral edge and a curved front surface. The tapered peripheral edge is preferably angled so as to provide a mechanical “overcut” and retain the thermoplastic blocking composition against the preformed base block. This avoids the need for adhesive

intermediate the thermoplastic blocking composition and the preformed base block. The blocking composition may be very easily and cleanly separated from the preformed base block by simply holding the preformed base and "peeling" the blocking composition off the base. Upon separation, very little if any blocking composition remains stuck to the preformed base. There is also no need to "dig" out blocking composition from cavities formed by "positively" tapered "undercuts". If desired, the cleanly separated preformed base block may then be reused, and the blocking composition recycled (i.e., reheated) and used again.

To prevent undesired rotation of the thermoplastic blocking composition relative to the preformed base block the preformed base block preferably also comprises a means to resist such rotation. This may be accomplished using an adhesive or a mechanical means. Suitable mechanical means include, for example, runners (e.g., off-centered fill holes) that extends at least partially through the preformed base block. Blocking composition that solidifies in the runner will help prevent such rotation. Alternatively, for example, the preformed base block may optionally comprise a non-circular periphery, such as a scalloped outer edge as shown in FIG. 9e or a key or plurality of keys as shown in FIG. 10e. Other mechanical means to resist rotation may be employed, if desired.

#### DETAILED DESCRIPTION OF THE DRAWINGS

Shown in FIG. 1 is an ophthalmic lens blank 10 and a conventional lens base block 20. A tape 12 or other lens coating is shown applied to the semi-finished surface of the lens and provides additional protection to keep the lens from being scratched or otherwise damaged by the heat of the lens blocking composition when the molten blocking composition is placed "adjacent" to the lens blank and/or to achieve better adherence between the base block and the lens blank. When base block 20 is placed against lens 10 a cavity is formed between cavity 21 of the block and the surface of the lens. A lens blocking composition may be injected through hole 22 to fill the cavity.

FIG. 2 depicts a side view of the ophthalmic lens blank 10 and lens base block 20 of FIG. 1. As shown in FIG. 2, an optional tape 12 or other lens coating may be applied to the semi-finished surface of the lens. A lens blocking composition 14 then fills the cavity formed between metal base block 20 and optional tape 12 on lens 10 and attaches the base block to the lens. Depending on the particular composition used, the composition may just fill the cavity or may form a film between the base block and the lens (as shown). FIG. 3 depicts an end view of the ophthalmic lens blank and lens block of FIG. 2. Base block 20 is provided with positioning guides 24 and hole 22 through which lens blocking composition 14 may be injected.

FIGS. 4a and 4b depict an alternative embodiment of the present invention wherein a lens block 16 is formed from the lens blocking composition of the present invention. If desired, a tape 12 or other lens coating may be first applied to the semi-finished surface of the lens. As shown in FIG. 4c, a mold 30 is used to define a cavity in the shape of a lens block. The mold 30 forms the cavity using the finished surface of lens 10 as one boundary. When a lens blocking composition is injected into the mold (e.g., through gate 26) and allowed to harden a rigid block is formed against and adhered to the lens or lens coating.

FIGS. 5a and 5b depict an alternative embodiment of the present invention wherein a lens block 16 is formed from the lens blocking composition of the present invention. If desired, a tape 12 or other lens coating may be first applied to the semi-finished surface of the lens 10. In this embodiment, lens block 16 comprises positioning guides 17 and hole 15.

FIGS. 6a and 6b depict a further alternative embodiment of the present invention wherein a lens block 16 is formed in part from the lens blocking composition of the present invention. In this embodiment, a preformed metal (or other rigid material) base block 25 is placed in the blocker, and the lens blocking composition is used to fill a cavity between the preformed base block and the lens 10 and to form a support ring of blocking composition against the lens. Preformed base block 25 may comprise one or more positioning guides 17, one or more polishing pin guide holes 24, and preferably contains an optional means to hold or "lock" the preformed base block against the blocker while the cavity is being filled with the blocking composition. One method for accomplishing this is to provide one or more "J-locks" 19, which engage pins on the blocker or on an optional cooling ring. The "J-locks" prevent the preformed base block from being pushed away from the blocker by the blocking composition. This ensured that the positioning guides of the preformed base will be in the desired alignment. Preformed base block 25 preferably contains a one or more holes 29 through its rear surface. When the base block and blocking composition are formed to provide a lens block, the blocking composition is viewable through the rear holes 29. After the block is separated from the lens, the user may conveniently separate the preformed base block from the blocking composition by holding the base block and pressing against the blocking composition (e.g., using a thumb or a tool) through the rear hole 29.

FIGS. 7a and 7b depict a further alternative embodiment of the present invention wherein a lens block 23 is formed in part from the lens blocking composition of the present invention. In this embodiment, a preformed metal (or other rigid material) base block 25 is placed in the blocker, and the lens blocking composition is used to fill the cavity between the preformed base block and the lens and to form a support ring of blocking composition against the lens. Preformed base block 25 may comprise one or more positioning guides 17, one or more polishing pin guide holes 24, and optionally contains a means to hold or "lock" the preformed base block against the blocker while the cavity is being filled with the blocking composition. Preformed base block 25 preferably contains a one or more holes 22 through its rear surface. When the base block and blocking composition are formed to provide a lens block, the blocking composition is viewable through the rear holes 22. After the block is separated from the lens, the user may conveniently separate the preformed base block from the blocking composition by holding the base block and pressing against the blocking composition (e.g., using a tool) through the rear surface hole 22.

Shown in FIG. 8a is an ophthalmic lens blank 10 and a lens block 40 of the present invention. The lens block 40 comprises a preformed base block 42 and a thermoplastic blocking composition 44. An optional tape 12 or other lens

coating is shown applied to the semi-finished surface of the lens 10 and provides additional protection to keep the lens 10 from being scratched or otherwise damaged by the heat of the lens blocking composition 44 when the molten blocking composition is placed "adjacent" to the lens blank and/or to achieve better adherence between the block and the lens blank. As shown in FIGS. 8b to 8d, preformed base block 42 is inserted into a mold 46 that is placed adjacent the lens blank 10. This forms a cavity between and optionally around at least a portion of the preformed base block 42 and the surface of the lens. The mold may also be fitted with a cooling apparatus, such as a water circuit 48 that allows the circulation of chilled water to pass. The thermoplastic blocking composition is then injected into the cavity between the preformed base block 42 and lens 10 and allowed to harden. The thermoplastic blocking composition 44 may be injected either through a hole 50 in the mold that is located opposite the lens (as shown in FIG. 8b and 8c) or through a hole 51 in the mold that is located on the side of the block 40 as is shown in FIG. 8d.

FIG. 8b depicts a side view of the ophthalmic lens blank 10 and lens block 40 of FIG. 1. As shown in FIG. 8b, an optional tape 12 or other lens coating may be applied to the semi-finished surface of the lens. A lens blocking composition 44 then fills the cavity formed between the mold 46, preformed base block 42, and lens 10; and attaches the preformed base block to the lens. FIG. 8c depicts a cross-sectional side view of the block 40 of FIGS. 8a and 8b. Preformed base block 42 is shown in FIG. 8f having a rear surface 54 and collar 55 that together are sized and adapted to fit the chuck of a desired lens processing machine. As such, the exact size and shape of this portion of the preformed base block may assume a variety of configurations. Preformed base block 42 preferably also has a "negatively" tapered edge 56 and a curved front surface 58. A fill hole 122 may optionally be provided through the preformed base block 42 to enable filling from the rear surface. Tapered edge 56 is preferably angled so as to provide a mechanical "overcut" and retain the thermoplastic blocking composition against the preformed base block 42. This avoids the need for adhesive between the thermoplastic blocking composition 44 and the preformed base block 42. The blocking composition may be very easily and cleanly separated from the preformed base block by simply holding the preformed base and "peeling" the blocking composition off the base. It has been observed that having a peripheral overcut retention means is preferred. Upon separation, very little if any blocking composition remains stuck to the preformed base. There is also no need to "dig" out blocking composition from cavities formed by "positively" tapered undercuts. If desired, the cleanly separated preformed base block may then be reused, and the blocking composition recycled (i.e., reheated) and used again. To prevent undesired rotation of the thermoplastic blocking composition 44 relative to the preformed base block 42 the preformed base block 42 preferably also comprises a means to resist such rotation. This may be accomplished using an adhesive or a mechanical means. For example, when the thermoplastic blocking composition is filled through an off-centered hole 122 that extends at least partially through the preformed base block, the material that solidifies in the hole will help prevent such

rotation. Alternatively, for example, the preformed base block may optionally comprise a scalloped outer edge 132 as shown in FIG. 9e or a key 140 or plurality of keys as shown in FIG. 10e. Other mechanical means to resist rotation may be employed, if desired.

FIGS. 8e to 8g illustrate the preformed base block of FIGS. 8a to 8c. FIG. 8e is a rear end view of preformed base block 42, showing positioning guides 117, polishing pin holes 124, fill hole 122, and outer edge 130. FIG. 8f is a side view of this same preformed base block 42, illustrating rear surface 54, collar 55, and tapered edge 56. FIG. 8g is a front end view of preformed base block 42, illustrating fill hole 122 and curved front surface 58. If desired, e.g., for preformed base blocks that are formed from a plastic material, the polishing pin guides optionally may be formed using a suitable insert, such as a metal or ceramic insert. The metal or ceramic inserts may resist wear that would compromise the polishing process.

FIGS. 9e to 9g illustrate an alternative embodiment of the preformed base block of FIGS. 8a to 8c. FIG. 9e is a rear end view of a preformed base block, showing positioning guides 117, polishing pin holes 124, and fill hole 122. The outer edge 132 in this example is scalloped so as to prevent rotation of the thermoplastic blocking composition about the preformed base block. FIG. 9f is a side view of this same preformed base block, illustrating rear surface 54, collar 55, and tapered edge 56. FIG. 9g is a front end view of this preformed base block, illustrating fill hole 122 and curved front surface 58.

FIGS. 10e to 10g illustrate a further alternative embodiment of the preformed base block of FIGS. 8a to 8c. FIG. 10e is a rear end view of a preformed base block, showing positioning guides 117, polishing pin holes 124, and fill hole 122. The outer edge 130 in this example contains at least one key 140 that helps prevent rotation of the thermoplastic blocking composition about the preformed base block. FIG. 10f is a side view of this same preformed base block, illustrating rear surface 54, collar 55, and tapered edge 56. FIG. 10g is a front end view of this preformed base block, illustrating fill hole 122 and curved front surface 58.

The following examples are offered to aid in the understanding of the present invention and are not to be construed as limiting the scope thereof. Unless otherwise indicated, all parts and percentages are by weight.

## EXAMPLES

### Example 1

Polyetherester block copolymers were synthesized by placing the reactants in the amounts listed in Table 1a into a 500 ml three-neck round bottom flask. The center neck had a stir shaft and paddle, one side neck had an adapter attached to a nitrogen source, and another side neck had a modified/Dean-Stark trap to condense and collect vapor. Run conditions for Runs 1-8 are given in Table 1b. The heat source was a Wood's metal bath commercially available from Aldrich Chemical Company, Milwaukee, Wis. The mixture was stirred with a nitrogen flow until it cooled to approximately 150° C. and then it was poured from the flask into a container.

TABLE 1a

| Reactants  |               |                  |                |            |                 |
|------------|---------------|------------------|----------------|------------|-----------------|
| Diacid     |               | Short Chain Diol |                | Polyol     |                 |
| Run Number | Name          | Amount (g)       | Name           | Amount (g) | Name            |
| 1          | succinic acid | 35.8             | 1,8-octanediol | 45.0       | TERETHANE™ 2900 |
| 2          | suberic acid  | 27.2             | 1,8-octanediol | 23.8       | TERETHANE™ 2900 |
| 3          | suberic acid  | 43.5             | 1,8-octanediol | 38.0       | TERETHANE™ 1000 |
| 4          | suberic acid  | 52.8             | 1,4-butanediol | 29.0       | TERETHANE™ 2900 |
| 5          | adipic acid   | 35.9             | 1,6-hexanediol | 31.2       | TERETHANE™ 2000 |
| 6          | suberic acid  | 32.9             | 1,4-butanediol | 18.9       | TERETHANE™ 2900 |
| 7          | suberic acid  | 52.8             | 1,4-butanediol | 29.2       | TERETHANE™ 1000 |
| 8          | succinic acid | 35.8             | 1,8-octanediol | 45.2       | TERETHANE™ 1000 |

<sup>1</sup>TERETHANE is the trademark for polyether glycols available from E. I. Du Pont de Nemours, Inc., Wilmington, DE.

TABLE 1b

| Run Conditions |                   |                             |
|----------------|-------------------|-----------------------------|
| Time (hours)   | Temperature (°C.) | Nitrogen Flow Rate (ml/min) |
| 0              | 150               | 100                         |
| 1              | 200               | 100                         |
| 4              | 240               | 500                         |
| 7 (Shut down)  | 150               | 500                         |

The polyetherester materials, Runs 1-3 and 5-8, and a competitive material, Comp. Run 9, commercially available as "FREE BOND™ Non-alloy Blocking Substance" from Gerber Optical Inc., South Windsor, Conn. were evaluated by Thermal Mechanical Analysis (TMA) using a "Perkin-Elmer 7 Series Thermal Analysis System" commercially available from The Perkin-Elmer Corporation, Norwalk, Conn. to determine the percent change in dimensions while heating over a temperature range of 0° C. to near the melting temperature at a rate of 5° C. per minute. An expansion probe with 50 mN of applied force was used. Transition temperatures and melting points were extrapolated at onset from the curves. The results for the polyetherester materials, Runs 1-3 and 5-8, and the competitive material, Comp. Run 9, are shown in Table 1c.

TABLE 1c

| Thermomechanical Analysis of Polyetheresters |                                                                    |                                                     |                                                 |
|----------------------------------------------|--------------------------------------------------------------------|-----------------------------------------------------|-------------------------------------------------|
| Run Number                                   | Percent Change in Dimensions for a Temperature Range (0° → 60° C.) | Extrapolated Onset of Transition Temperatures (°C.) | Extrapolated Onset of Melting Temperature (°C.) |
| 1                                            | 1.6 (0° → 60° C.)                                                  | 39, 55                                              | 64                                              |
| 2                                            | 2.8 (0° → 52° C.)                                                  | 32, 19, 19, 20                                      | 57                                              |
| 3                                            | 1.7 (0° → 60° C.)                                                  | 40, 38, 39                                          | 62                                              |
| 5                                            | 1.5 (0° → 45° C.)                                                  | 26                                                  | 48                                              |
| 6                                            | 2.2 (0° → 45° C.)                                                  | 29, 17, 17                                          | 47                                              |
| 7                                            | 1.7 (0° → 49° C.)                                                  | 34, 36, 37                                          | 50                                              |
| 8                                            | 1.5 (0° → 58° C.)                                                  | 34, 34, 34                                          | 60                                              |

20

TABLE 1c-continued

| Run Number  | Thermomechanical Analysis of Polyetheresters             |                               |                           |
|-------------|----------------------------------------------------------|-------------------------------|---------------------------|
|             | Percent Change in Dimensions for a Temperature Range (%) | Transition Temperatures (°C.) | Melting Temperature (°C.) |
| Comp. Run 9 | 2.9 (0° → 41° C.)                                        | 29, 25, 26                    | 44                        |

25

The polyetherester materials, Runs 1-3 and 5-8 had higher melting temperatures and a lower percent change in dimensions over the temperature range of heating than the competitive material in Comp. Run 9.

The polyetherester materials, Runs 1-8, were evaluated by Gel Permeation Chromatography (GPC) for weight, number, and z average molecular weights. GPC analysis was done in tetrahydrofuran (THF) at 1.0 ml/min. using a 40 HP1090LC System from Hewlett-Packard, Palo Alto, Calif. including a HP 1047A Refractive Index detector and a HP Diode Array Detector (UV detector at 254 nm). A CRI Permagel 10 micron particle size column from Column Resolutions Inc., San Jose, Calif. was used for high molecular weight materials. Analog signals were converted to digital data using Polymer Laboratories, Inc., Amherst, Mass., software and hardware. Calibration was based on polystyrene standards from Pressure Chemical Co., Pittsburgh, Pa. The sample solution was weighed accurately to give 15 mg of resin/5 ml solvent and filtered with a 0.2 micron "TEFLON™ Filter" from Scientific Resources, Eatontown, N.J. and 100 microliters was injected into the column. A Polydispersity Index was calculated by dividing  $M_w$  by  $M_n$ . The results are shown in Table 1d.

30

35

40

45

50

55

TABLE 1d

| Run Number | Weight Average Molecular Weight ( $M_w$ ) | Number Average Molecular Weight ( $M_n$ ) | Z Average Molecular Weight ( $M_z$ ) | Polydispersity Index ( $M_w/M_n$ ) |
|------------|-------------------------------------------|-------------------------------------------|--------------------------------------|------------------------------------|
| 1          | 23684                                     | 9871                                      | 38973                                | 2.40                               |
| 2          | 21411                                     | 10554                                     | 34580                                | 2.03                               |
| 3          | 15015                                     | 7253                                      | 24074                                | 2.07                               |
| 4          | 21488                                     | 8682                                      | 35976                                | 2.48                               |
| 5          | 16403                                     | 4816                                      | 28342                                | 3.41                               |
| 6          | 21066                                     | 11826                                     | 31237                                | 1.78                               |

TABLE 1d-continued

| Run Number | Weight Average Molecular Weight (M <sub>w</sub> ) | Number Average Molecular Weight (M <sub>n</sub> ) | Z Average Molecular Weight (M <sub>z</sub> ) | Polydispersity Index (M <sub>w</sub> /M <sub>n</sub> ) |
|------------|---------------------------------------------------|---------------------------------------------------|----------------------------------------------|--------------------------------------------------------|
| 7          | 18119                                             | 9199                                              | 28880                                        | 1.97                                                   |
| 8          | 15448                                             | 7973                                              | 23949                                        | 1.94                                                   |

Number average molecular weight equals weight average molecular weight for a monodisperse system. Polydispersity Index is a measure of the breadth of the polymer molecular weight distribution. Run 5 had the broadest molecular weight distribution.

The flow behavior of polyetherester formulations was examined using a parallel plate fixture on a Rheometrics Dynamic Analyzer (RDA-II) from Rheometrics, Inc., Piscataway, N.J. The steady shear viscosity (Pa s) was measured at shear rates of 1, 5, and 10 second<sup>-1</sup> at 65.6° C. At each shear rate, the measurement was made when the torque was at steady state. The results are shown in Table 1e.

TABLE 1e

| Run Number  | Shear Viscosity at Shear Rates of 1, 5, and 10 second <sup>-1</sup> (Pa s) |                   |                    |
|-------------|----------------------------------------------------------------------------|-------------------|--------------------|
|             | 1 s <sup>-1</sup>                                                          | 5 s <sup>-1</sup> | 10 s <sup>-1</sup> |
| 1           | 15.27                                                                      | 15.11             | 15.16              |
| 2           | 7.45                                                                       | 7.44              | 7.39               |
| 3           | 3.16                                                                       | 3.04              | 3.02               |
| 5           | 5.22                                                                       | 5.16              | 5.17               |
| 6           | 9.93                                                                       | 9.59              | 9.67               |
| 7           | 5.37                                                                       | 5.36              | 5.37               |
| 8           | 3.44                                                                       | 3.83              | 3.86               |
| Comp. Run 9 | 0.98                                                                       | 0.91              | 0.88               |

The differences in the measured viscosity indicated variation in the molecular weight of the resin systems. For the "FREE BOND™ Non-alloy Blocking substance" (Comp. Run 9), the measured viscosity was at the limit of the instrument sensitivity; therefore, the viscosity may be approximate values.

The polyetherester materials, Runs 1–3 and 5–8, and the competitive material, Comp. Run 9, were evaluated for hardness using ASTM Test Method D2240-91 "Shore Type 'A' Hardness". Three measurements were made for each run. The results are shown in Table 1f.

TABLE 1f

| Run Number  | Shore Type 'A' Hardness Test (ASTM D2240-91) Measurement |    |    |         |
|-------------|----------------------------------------------------------|----|----|---------|
|             | 1                                                        | 2  | 3  | Average |
| 1           | 96                                                       | 97 | 93 | 95      |
| 2           | 93                                                       | 96 | 96 | 95      |
| 3           | 78                                                       | 77 | 78 | 78      |
| 5           | 46                                                       | 43 | 39 | 43      |
| 6           | 83                                                       | 83 | 83 | 83      |
| 7           | 82                                                       | 79 | 84 | 82      |
| 8           | 81                                                       | 79 | 81 | 80      |
| Comp. Run 9 | 66                                                       | 63 | 64 | 64      |

## Example 2

Polycaprolactone materials commercially available as "TONE™ P-300" (10,000 molecular weight) polycaprolactone

from Union Carbide Chemicals and Plastics Company Inc., Danbury, Conn., Run 1, and as "CAPA™ 630" (30,000 molecular weight) polycaprolactone from Solvay Interox, Houston, Tex., Run 2, were evaluated by Thermal Mechanical Analysis (TMA) using the same procedure described for Example 1. The results are shown in Table 2a along with the results of two comparison runs.

TABLE 2a

| Run Number               | Percent Change in Dimensions for a Temperature Range | Extrapolated Onset of         |                           |
|--------------------------|------------------------------------------------------|-------------------------------|---------------------------|
|                          |                                                      | Transition Temperatures (°C.) | Melting Temperature (°C.) |
| 1                        | 1.0 (0°→54° C.)                                      | 41, 47                        | 61                        |
| 2                        | 1.4 (0°→54° C.)                                      | 26, 38, 41                    | 60                        |
| Comp. Run 3 <sup>1</sup> | 1.9 (0°→40° C.)                                      |                               | 46                        |
| Comp. Run 4 <sup>2</sup> | 2.9 (0°→41° C.)                                      | 29, 25, 26                    | 44                        |

<sup>1</sup>"OPTEK™ Feather Lite Blocking Compound" available from Associated Development Corporation, Optek Division, Pinellas Park, FL.

<sup>2</sup>"FREE BOND™ Non-alloy Blocking Substance" available from Gerber Optical Inc., South Windsor, CT.

The polycaprolactone materials, Runs 1 and 2, had a higher melt temperature and a lower percent change in dimensions over a temperature range of heating than the competitive materials in Comp. Runs 3 and 4.

The polycaprolactone materials and the two comparison materials were evaluated by Gel Permeation Chromatography (GPC) for weight, number, and z average molecular weights using the same procedure described for Example 1. The results are shown in Table 2b.

TABLE 2b

| Run Number      | Weight Average Molecular Weight (M <sub>w</sub> ) | Number Average Molecular Weight (M <sub>n</sub> ) | Z Average Molecular Weight (M <sub>z</sub> ) | Polydispersity Index (M <sub>w</sub> /M <sub>n</sub> ) |
|-----------------|---------------------------------------------------|---------------------------------------------------|----------------------------------------------|--------------------------------------------------------|
| 1a              | 23850                                             | 5220                                              | 38803                                        | 4.57                                                   |
| 1b <sup>1</sup> | 23520                                             | 4720                                              | 38611                                        | 4.98                                                   |
| 2               | 61800                                             | 40190                                             | 87281                                        | 1.54                                                   |
| Comp. Run 3     | 35470                                             | 2500                                              | 179460                                       | 14.18                                                  |
| Comp. Run 4     | 26570                                             | 1140                                              | 172450                                       | 23.35                                                  |

<sup>1</sup>Run 1b differed from Run 1a in that this sample was aged in an oven at 66° C. for 30 days before GPC testing.

The polydispersity index shows that the competitive blocking compounds, Comp. Runs 3 and 4 had very broad molecular weight distributions. The "TONE™ P-300 Polycaprolactone" from Union Carbide Chemicals and Plastics Company Inc., Runs 1a and 1b had a somewhat broader molecular weight distribution than "CAPA™ 630 Polycaprolactone" from Solvay Interox, Run 2.

The flow behavior of polycaprolactone materials, Runs 1 and 2, and the two comparison materials, Comp. Runs 3 and 4, were examined using the same procedure described for Example 1. The results are shown in Table 2c.

TABLE 2c

| Run Number  | Shear Viscosity<br>at Shear Rates of 1, 5, and 10 second <sup>-1</sup> (Pa s) |                   |                    |
|-------------|-------------------------------------------------------------------------------|-------------------|--------------------|
|             | 1 s <sup>-1</sup>                                                             | 5 s <sup>-1</sup> | 10 s <sup>-1</sup> |
| 1           | 15.5                                                                          | 15.6              | 15.7               |
| 2           | 407.3                                                                         | 408.9             | 410.0              |
| Comp. Run 3 | 2.6                                                                           | 2.4               | 2.21               |
| Comp. Run 4 | 0.98                                                                          | 0.91              | 0.88               |

The polycaprolactone materials, Runs 1 and 2, had a higher viscosity than the competitive materials in Comp. Runs 3 and 4. The polycaprolactone in Run 2 had a significantly higher viscosity than any of the other materials.

The tangent modulus of elasticity in bending and flexural strength were measured for the two polycaprolactones and the competitive materials using ASTM D 790-86, "Standard Test Methods for Flexural Properties of Unreinforced and Reinforced Plastics and Electrical Insulating Materials" Test Method I. This test employs a three-point loading system utilizing center loading on a simply supported beam. The specimen were molded by heating the material to its melting temperature and pouring into a fluorocarbon coated mold die to give a test specimen that was 165 mm long, 12 mm wide, and 6 mm thick. The measurements were made on a "MTS SinTech™ Mechanical Tester" from MTS Systems Corporation, Eden Prairie, Minn. The span tested was 96 mm long giving a span to depth ratio equal to 16:1. The crosshead motion was 2 mm per min. Four specimen were tested for each Run. The results are shown in Tables 2d and 2e.

TABLE 2d

| Run Number  | Tangent Modulus of Elasticity in Bending<br>(ASTM D790-86)<br>(MPa) |     |     |     |      |                    |
|-------------|---------------------------------------------------------------------|-----|-----|-----|------|--------------------|
|             | 1                                                                   | 2   | 3   | 4   | Mean | Standard Deviation |
| 1           | 355                                                                 | 367 | 313 | 256 | 323  | 50                 |
| 2           | 408                                                                 | 224 | 355 | 266 | 313  | 83                 |
| Comp. Run 3 | 28                                                                  | 48  | 32  | 11  | 30   | 15                 |
| Comp. Run 4 | 30                                                                  | 22  | 29  | 37  | 29   | 6                  |

The polycaprolactone materials in Runs 1 and 2 had ten times greater bending modulus than the comparison competitive materials in Runs 3 and 4.

TABLE 2e

| Run Number  | Flexural Strength (ASTM D790-86)<br>(MPa) |      |      |      |      |                    |
|-------------|-------------------------------------------|------|------|------|------|--------------------|
|             | 1                                         | 2    | 3    | 4    | Mean | Standard Deviation |
| 1           | 2.7                                       | 2.8  | 3.0  | 2.0  | 2.6  | 0.3                |
| 2           | 14.3                                      | 13.3 | 20.1 | 18.1 | 16.5 | 3.2                |
| Comp. Run 3 | 0.5                                       | 1.3  | 0.7  | 0.7  | 0.8  | 0.4                |
| Comp. Run 4 | 1.2                                       | 0.8  | 0.7  | 1.2  | 1.0  | 0.3                |

The polycaprolactone used in Run 2 had a flexural strength that was six times greater than the polycaprolactone used in Run 1 and fifteen times greater than the comparison competitive materials in Comp. Runs 3 and 4. As a result of having greater rigidity, the polycaprolactone materials should exhibit less flexing during normal lens processing conditions.

## Hardness Test

The hardness of the polycaprolactone materials used in Run 1 and 2 and the competitive materials in Comp. Runs 3 and 4 was determined using a nanoindentation method. An ultramicro hardness tester, "UMIST™ 2000 Tester" from Division of Applied Physics, CSIRO, Australia was used. A Berkovich diamond indenter with a cone angle of 65 degrees was impressed against a surface in load increments of 1 mN while the resultant displacement was measured until the maximum load of 60 mN was achieved, then the load was incrementally decreased at 1 mN and the material's elastic recovery was observed as a decrease in total penetration. The hardness is equal to maximum load divided by the projected area of plastic deformation (i.e. contact area) and is reported in giga-pascals (GPa). The results are shown in Table 2f.

TABLE 2f

| Run Number  | Hardness<br>(GPa) |
|-------------|-------------------|
| 1           | 5.02              |
| 2           | 5.29              |
| Comp. Run 3 | 0.00187           |
| Comp. Run 4 | 0.14              |

The polycaprolactones, Runs 1 and 2, were significantly harder than the competitive materials, Comp. Runs 3 and 4.

## Probe Tack Test

A probe tack test was used to evaluate the tackiness of the materials and is described in ASTM D2979-88. Aluminum tins, 57 mm in diameter, were tared and three grams of each polycaprolactone (Runs 1 and 2) and each competitive material (Comp. Runs 3 and 4) were added to a tin. The materials were melted on a standard hot plate and cooled for 2 minutes. A 25.4 mm by 25.4 mm square of the material including the aluminum beneath the material was scissors cut and placed on the test probe area of a "TMI Polyken Probetack (Model 80-02-01)" commercially available from Testing Machines Inc., Amityville, N.Y. with an "A" annular weight of 200 grams (foam side down) on top of the aluminum side of the sample and the material side directly on top of the test probe. The machine settings were: Speed—0.5 cm; Dwell time: 2 seconds; Mode: peak. The test was initiated and the peak value recorded in grams. The results are shown in Table 2g.

TABLE 2g

| Run Number  | 1<br>(g) | 2<br>(g) | 3<br>(g) | 4<br>(g) | 5<br>(g) | Mean<br>tack<br>(g) | Standard<br>Deviation<br>(g) |
|-------------|----------|----------|----------|----------|----------|---------------------|------------------------------|
| 1           | 213      | 290      | 313      | 290      | 271      | 275                 | 38                           |
| 2           | 364      | 481      | 267      | 325      | 38       | 364                 | 79                           |
| Comp. Run 3 | 115      | 109      | 110      | 90       | 102      | 105                 | 10                           |
| Comp. Run 4 | 1190     | 1462     | 1474     | 1090     | 1067     | 1257                | 198                          |

The probe tack test showed that "FREE BOND™ Non-alloy Blocking Substance" (Comp. Run 4) was significantly stickier than the polycaprolactone materials (Runs 1 and 2) and "OPTIK™ Feather Lite Blocking Compound" (Comp. Run 3). Thus, "FREE BOND™ Non-alloy Blocking Substance" would be stickier around the laboratory and more difficult to clean from surfaces.

## Shear Adhesion Test

Circular polymethacrylate resin mounts were made and then ground using Grade 120 silicon carbide paper-backed

abrasive mounted on a lapidary wheel. Further grinding and polishing of the mounts was carried out by mounting Grade 600 silicon carbide paper-backed abrasive on the lapidary wheel. Approximately 2.8 cm circles were cut from each of two commercially available tapes: A) "VENTURE™ Tape", available from Venture Tape Corp., Rockland, Mass.; and B) "SURFACE SAVER™ #1640 Lens Surface Systems" available from 3M Company, St. Paul, Minn. The tape circles were applied to the resin mounts with the adhesive side of the tape on the smooth surface of the resin mount, rolled twice with a two inch hand roller, and placed on a round 0.5 cm mold made from a 2 mm thick "TEFLON™ Polytetrafluoroethylene Sheet" with a 5 mm diameter circular hole through the sheet. The hole in each mold was filled using syringes with melted polycaprolactone from Run 1 or 2, competitive materials from Comparison Runs 3 or 4, or a low-melting-temperature blocking alloy commercially available as "Coburn Blok-alloy 9916" from Coburn Optical Industries, Muskogee, Okla., Comp. Run 5. The materials were allowed to harden and the mold was removed leaving resin mounts with the applied tape sample molded to the polycaprolactone, competitive materials or blocking alloy.

Adhesive strength was evaluated by mounting the resin mount in a holder clamped in the jaws of an "INSTRON™ Testing Apparatus" with the polished mount surface oriented parallel to the direction of pull. A loop of 0.44 mm diameter wire was placed around the base of the hardened materials. The ends of the wire were clamped in the pulling jaw of the tensile testing apparatus, placing the bond in shear stress. The bond was stressed until it failed, using a crosshead speed of 2 mm/min. Shear adhesion values for 10 samples of each material were measured and the average and standard deviation recorded. The results are recorded in Table 2h.

The temperature was progressively increased from 177° C. to 277° C. from zone 1 to zone 3. The die temperature was 288° C.

A double coated tape commercially available as "3M Double Coated 1512 Tape" was applied to one side of the backing layer of the lens surface protective film and to 70 mm plastic lenses with 2.0–2.4 mm center thickness, plano, finished uncut, "RLX Plus™ Scratch Resistant, Finished Lens in Hard Resin" from Signet Armorlite, Inc., San Marcos, Calif. using the 3M SURFACE SAVER Applicator available from 3M. Air pressure was set at 0.02–0.03 MPa for the blocker commercially available as OPTEK™ Model 200 Blocker. A brass blocking ring was placed on the blocker and a 56 mm diameter Coburn Block from Coburn Company was placed into the ring such that the inlet in the block fit snugly over the rubber nozzle. The block was centered on the lens and slowly filled with polycaprolactone from Run 1 at 60° C. The blocked lens assembly was allowed to set for 10 to 15 seconds after filling, in order for the resin to harden and form a good bond to the taped lens. The blocking ring and blocked lens was removed from the blocker and the blocked lens was removed from the blocking ring.

The heat transfer temperature of the melted polycaprolactone was measured at the lens surface using a temperature probe sandwiched between the lens surface and the adhesive side of the surface protector tape. The results are shown in Table 2i.

TABLE 2h

| Shear Adhesion Test               |                             |                                                     |                |                                          |                |                                        |  |
|-----------------------------------|-----------------------------|-----------------------------------------------------|----------------|------------------------------------------|----------------|----------------------------------------|--|
| Number Bonded out of 10 specimens |                             | Average adhesion value (kg/cm <sup>2</sup> )        |                | Standard Deviation (kg/cm <sup>2</sup> ) |                |                                        |  |
| Run Number                        | "VENTURE Tape" <sup>1</sup> | "SURFACE SAVER Lens Surfacing Systems" <sup>2</sup> | "VENTURE Tape" | "SURFACE SAVER Lens Surfacing Systems"   | "VENTURE Tape" | "SURFACE SAVER Lens Surfacing Systems" |  |
| 1                                 | 10                          | 10                                                  | 8.15           | 18.12                                    | 1.66           | 1.61                                   |  |
| 2                                 | 0                           | 10                                                  | —              | Tape Ripped                              | —              | —                                      |  |
| Comp. Run 3                       | 0                           | 2                                                   | —              | 4.51                                     | —              | 1.14                                   |  |
| Comp. Run 4                       | 3                           | 4                                                   | 5.56           | 6.25                                     | 2.44           | 1.17                                   |  |
| Comp. Run 5                       | 2                           | 10                                                  | 12.15          | 12.96                                    | 4.09           | 2.80                                   |  |

<sup>1</sup>"VENTURE™ No. 455 Tape" commercially available from Venture Tape Corp., Rockland, MA

<sup>2</sup>"SURFACE SAVER™ #1640 Lens Surfacing Systems" commercially available from 3M Company, St. Paul, MN

#### Lens Distortion Test

A surface protection tape was made by blending two resins, "BYNEL™ 3101 Acid and Acrylate Modified Ethylene Vinyl Acetate" (25 wt. %) from E. I. Du Pont de Nemours and Company, Wilmington, Del. and "ATTANE™ 4602 Ultra Low Density Ethylene/Octene Copolymer" (75 wt. %) from Dow Chemical Company, Midland, Mich. on a "Haake Rheocord extruder" (Model 252) commercially available from Haake Inc., Saddle Brook, N.J. with a 1.9 cm diameter screw and with a length to diameter (L:D) ratio of 25:1 to form the backing layer of the surface protection tape.

TABLE 2i

| Time (minutes) | Temperature (°C.) |
|----------------|-------------------|
| 0              | 25.56             |
| 1              | 36.67             |
| 2              | 36.11             |
| 3              | 36.11             |
| 4              | 36.11             |
| 5              | 35.56             |

TABLE 2i-continued

| Time (minutes) | Temperature (°C.) |
|----------------|-------------------|
| 6              | 35.00             |
| 7              | 34.44             |
| 8              | 34.44             |
| 9              | 33.89             |
| 10             | 33.89             |
| 11             | 33.89             |
| 12             | 33.89             |
| 13             | 33.89             |
| 14             | 33.33             |
| 15             | 33.33             |
| 16             | 33.33             |

The lens were examined and found to be distortion "free" which means that it is safe to block such lenses with a surface protector tape at 60° C.

#### Cooling Rates

The cooling rates of the polycaprolactones, Runs 1 and 2, were compared to the blocking alloy commercially available as "Coburn Blok-alloy 9916" from Coburn Optical Industries, Comp. Run 5 and the competitive material used in Comp. Run 4. An Omega Model HH21 microprocessor thermometer type J-K-T thermocouple was placed below the tape and against the lens. The results are shown in Table 2j.

TABLE 2j

| Time<br>(Minutes) | Temperature (°C.) |       |             |             |
|-------------------|-------------------|-------|-------------|-------------|
|                   | Run 1             | Run 2 | Comp. Run 4 | Comp. Run 4 |
| 1                 | 66.67             | 67.22 | 65.56       | 66.67       |
| 2                 | 62.78             | 63.89 | 62.22       | 61.67       |
| 3                 | 63.33             | 61.11 | 57.78       | 57.22       |
| 4                 | 58.89             | 58.89 | 55.56       | 53.89       |
| 5                 | 56.67             | 56.67 | 52.78       | 50.56       |
| 6                 | 52.78             | 54.44 | 47.78       | 47.78       |
| 7                 | 50.00             | 53.33 | 45.00       | 45.56       |
| 8                 | 50.00             | 51.67 | 43.33       | 44.44       |
| 9                 | 48.33             | 50.00 | 38.33       | 43.89       |
| 10                | 46.67             | 48.33 | 40.00       | 45.00       |
| 11                | 44.44             | 46.67 | 38.89       | 45.00       |
| 12                | 43.89             | 45.36 | 37.78       | 45.00       |
| 13                | 42.78             | 43.89 | 36.11       | 45.00       |
| 14                | 41.67             | 42.78 | 36.11       | 45.00       |
| 15                | 40.56             | 41.67 | 35.56       | 45.00       |
| 20                | 38.89             | 37.78 | 33.33       | 45.00       |
| 25                | 40.00             | 37.78 | 31.11       | 45.00       |
| 30                | 40.00             | 38.33 | 30.00       | 45.56       |
| 35                | 37.78             | 37.78 | 28.89       | 45.56       |
| 40                | 32.78             | 37.22 | 27.22       | 45.56       |
| 45                | 31.67             | 36.67 | 26.67       | 45.56       |
| 50                | 31.11             | 35.00 | 26.11       | 43.89       |
| 55                | 28.89             | 33.33 | 25.00       | 36.67       |
| 60                | 27.22             | 27.22 | 25.00       | 31.11       |
| 65                | 27.78             | 27.78 | 25.00       | 28.33       |
| 70                | 28.89             | 28.89 | 25.00       | 27.78       |

Blocking alloy, Comp. Run 5, initially cooled faster than any of the other materials in the first five minutes and then after ten minutes it held at a temperature between 45.00° C. and 45.56° C. which was a slower cooling rate. "FREE BOND™ Non-alloy Blocking Substance", Comp. Run 4, cooled more quickly than any of the other materials.

#### Example 3

Low molecular weight polycaprolactones commercially available as "TONE™ Polyol 1270" (reported MW=4,000), "TONE™ Polyol 0260" (reported MW=3,000), and "TONE™ Polyol 2241" (reported MW=2,000) from Union

Carbide Chemicals and Plastics Company Inc., Danbury, Conn. were blended with a higher molecular weight poly-caprolactone (PCL) commercially available as "TONE™ Polyol P-300" (reported MW=10,000) from Union Carbide 5 Chemicals and Plastics Company Inc. in the amounts shown in Table 3a, Runs 1-12. The polycaprolactones were placed in a high density polyethylene container in an oven at 65° C. until they were melted, approximately 2 hours. The container was placed in boiling water on a hot plate with a mechanical stirrer for a few minutes. The container was returned to a 65° C. oven to deaerate the molten polymers. Then the molten polymers were poured onto a tray to cool to room temperature and solidify. Low molecular weight 10 polycaprolactone triols (reported MW=300, 530, and 1250) 15 commercially available from Aldrich Chemical Co., Inc., Milwaukee, Wis. were added to the melt of the higher molecular weight polycaprolactone, Run 1, in varying amounts (Table 3a) in Runs 13-24.

Hardness was measured using two durometers commercially 20 available as Model 307L for Shore Type 'D' and Model 306L for Shore Type 'A' from Pacific Transducer 25 Corporation, Los Angeles, Calif. according to ASTM D2240-91.

Viscosity of the molten polymer mixtures were determined 30 using a Brookfield viscometer, Model LVT, spindle No. 34 commercially available from Brookfield Engineering Laboratories, Inc., Stoughton, Mass. at 60° C. The spindle end was immersed to about 0.6 cm in the melt and readings were taken at intervals for 5 to 10 minutes until the reading was constant. The viscosity in centipoise (cP) was calculated.

TABLE 3a

| Run<br>Number | High<br>Molecular<br>Weight PCL <sup>1</sup><br>(wt. %) | Low<br>Molecular<br>Weight<br>PCL <sup>1</sup><br>(wt. %) | Low<br>Molecular<br>Weight<br>PCL Triol<br>(wt. %) | Hardness<br>Shore<br>'D'/'A' | Viscosity<br>(cP) |                   |
|---------------|---------------------------------------------------------|-----------------------------------------------------------|----------------------------------------------------|------------------------------|-------------------|-------------------|
|               |                                                         |                                                           |                                                    |                              | Run<br>Number     | Viscosity<br>(cP) |
| 1             | 100                                                     | 0                                                         | 0                                                  | 53/98                        | 23000             |                   |
| 2             | 80                                                      | 20 <sup>2</sup>                                           | 0                                                  | 52/98                        | 14800             |                   |
| 3             | 60                                                      | 40 <sup>2</sup>                                           | 0                                                  | 47/98                        | 10600             |                   |
| 4             | 40                                                      | 60 <sup>2</sup>                                           | 0                                                  | 47/98                        | 8000              |                   |
| 5             | 20                                                      | 80 <sup>2</sup>                                           | 0                                                  | 40/—                         | 2600              |                   |
| 6             | 0                                                       | 100 <sup>2</sup>                                          | 0                                                  | 46/98                        | 11600             |                   |
| 7             | 80                                                      | 20 <sup>3</sup>                                           | 0                                                  | 42/98                        |                   |                   |
| 8             | 60                                                      | 40 <sup>3</sup>                                           | 0                                                  |                              |                   |                   |
| 9             | 0                                                       | 100 <sup>3</sup>                                          | 0                                                  |                              |                   | 1500              |
| 10            | 80                                                      | 20 <sup>4</sup>                                           | 0                                                  | 44/98                        | 11200             |                   |
| 11            | 60                                                      | 40 <sup>4</sup>                                           | 0                                                  | 40/96                        | 5400              |                   |
| 12            | 0                                                       | 100 <sup>4</sup>                                          | 0                                                  | 15/80                        | 450               |                   |
| 13            | 90                                                      | 0                                                         | 10 <sup>5</sup>                                    | 50/—                         | 15000             |                   |
| 14            | 80                                                      | 0                                                         | 20 <sup>5</sup>                                    | 42/—                         | 10800             |                   |
| 15            | 0                                                       | 0                                                         | 100 <sup>5</sup>                                   |                              | 90                |                   |
| 16            | 97.5                                                    | 0                                                         | 2.5 <sup>6</sup>                                   |                              | 18400             |                   |
| 17            | 95                                                      | 0                                                         | 5 <sup>6</sup>                                     | 40/98                        | 15400             |                   |
| 18            | 90                                                      | 0                                                         | 10 <sup>6</sup>                                    | 30/—                         |                   |                   |
| 19            | 80                                                      | 0                                                         | 20 <sup>6</sup>                                    | 30/—                         |                   |                   |
| 20            | 70                                                      | 0                                                         | 30 <sup>6</sup>                                    | 30/—                         |                   |                   |
| 21            | 95                                                      | 0                                                         | 5 <sup>7</sup>                                     | 40/98                        |                   |                   |
| 22            | 90                                                      | 0                                                         | 10 <sup>7</sup>                                    | 30/—                         |                   |                   |

TABLE 3a-continued

| Run Number | High Molecular Weight PCL <sup>1</sup><br>(wt. %) | Low Molecular Weight PCL <sup>1</sup><br>(wt. %) | Low Molecular Weight PCL Triol <sup>2</sup><br>(wt. %) | Hardness 'D'/'A' <sup>5</sup> | Viscosity (cP) |
|------------|---------------------------------------------------|--------------------------------------------------|--------------------------------------------------------|-------------------------------|----------------|
| 23         | 80                                                | 0                                                | 20 <sup>7</sup>                                        | 30/—                          |                |
| 24         | 70                                                | 0                                                | 30 <sup>7</sup>                                        | 30/—                          |                |

<sup>1</sup>“TONE™ Polyol P-300” polycaprolactone available from Union Carbide Chemicals and Plastics Company, Inc., Danbury, CT

<sup>2</sup>“TONE™ Polyol 1270” polycaprolactone available from Union Carbide Chemicals and Plastics Company, Inc.

<sup>3</sup>“TONE™ Polyol 0260” polycaprolactone available from Union Carbide Chemicals and Plastics Company, Inc.

<sup>4</sup>“TONE™ Polyol 2241” polycaprolactone available from Union Carbide Chemicals and Plastics Company, Inc.

<sup>5</sup>Low molecular weight polycaprolactone triol (reported MW = 1250) commercially available from Aldrich Chemical Co., Inc., Milwaukee, WI

<sup>6</sup>Low molecular weight polycaprolactone triol (reported MW = 530) commercially available from Aldrich Chemical Co., Inc.

<sup>7</sup>Low molecular weight polycaprolactone triol (reported MW = 300) commercially available from Aldrich Chemical Co., Inc.

spheres were placed in a HDPE container in an oven at 65° C. until the polycaprolactone was melted. Then the container was placed in boiling water on a hot plate with a mechanical stirrer for a few minutes. The container was placed back in a 65° C. oven to deaerate. The molten polymer mixture was poured into an anodized aluminum metal block commercially available from Coburn, Muskogee, Okla., covered with a polyethylene film, and molded in a concave shape. The block was cooled and the polycaprolactone mixture solidified. The melting time was evaluated by observing the time in seconds that the polymer mixture took to melt at 65° C. under a 500 watt GE sun lamp held at a distance of 125 mm from the surface of the polymer.

The polycaprolactone mixtures were also evaluated for hardness. The results are shown in Table 4a. Hardness was measured using ASTM D2240-91 “Shore Type ‘D’”.

TABLE 4a

| Run Number | PCL (wt. %)      | Inorganic pigment <sup>3</sup> (wt. %) | Carbon Black <sup>4</sup> (wt. %) | Ceramic Microspheres <sup>5</sup> (wt. %) | Melting Time (seconds) | Hardness Shore ‘D’ |
|------------|------------------|----------------------------------------|-----------------------------------|-------------------------------------------|------------------------|--------------------|
| 1          | 100 <sup>1</sup> | 0                                      | 0                                 | 0                                         | >120                   | 53                 |
| 2          | 95 <sup>1</sup>  | 5                                      | 0                                 | 0                                         | 10–15                  | 54                 |
| 3          | 90 <sup>1</sup>  | 10                                     | 0                                 | 0                                         | 10–15                  | 57                 |
| 4          | 95 <sup>1</sup>  | 0                                      | 5                                 | 0                                         | 10–15                  | 53                 |
| 5          | 90 <sup>1</sup>  | 0                                      | 10                                | 0                                         | 10–15                  | 53                 |
| 6          | 80 <sup>2</sup>  | 0                                      | 0                                 | 20                                        | 10                     | 45                 |
| 7          | 100 <sup>2</sup> | 0                                      | 0                                 | 0                                         | >60                    | 40                 |

<sup>1</sup>“TONE™ Polyol P-300” polycaprolactone available from Union Carbide Chemicals and Plastics Company, Inc., Danbury, CT

<sup>2</sup>“TONE™ Polyol 1270” polycaprolactone available from Union Carbide Chemicals and Plastics Company, Inc.

<sup>3</sup>“F-6331” black inorganic pigment available from Ferro Corporation, Color Division, Cleveland, OH

<sup>4</sup>“AROSPHERE 11” carbon black available from Huber Corporation, Borger, TX

<sup>5</sup>“ZEEOSPHERES™ Z-200” ceramic microspheres available from 3M Company, St. Paul, MN

The addition of lower molecular weight solid polycaprolactone in Runs 2–12 helped to reduce the viscosity of the blend. The addition of low molecular weight polycaprolactone triol in Runs 13–24 served as a plasticizer making the polycaprolactone blend soft while decreasing viscosity.

#### Example 4

Carbon black commercially available as “AROSPHERE 11” from Huber Corp., Borger, Tex. and a black inorganic pigment commercially available as “F-6331” from Ferro Corporation, Color Division, Cleveland, Ohio were added in the amounts shown in Table 4a to a polycaprolactone commercially available as “TONE™ Polyol P-300” (10,000 molecular weight) from Union Carbide Chemicals and Plastics Company, Inc. Ceramic microspheres commercially available as “ZEEOSPHERES™ 200” from 3M Company, St. Paul, Minn. were added in the amounts shown in Table 4a to a polycaprolactone commercially available as “TONE™ Polyol 1270” (4,000 molecular weight) from Union Carbide Chemicals and Plastics Company, Inc. The polycaprolactone and carbon black, pigment, or micro-

50 spheres were placed in a HDPE container in an oven at 65° C. until the polycaprolactone was melted. Then the container was placed in boiling water on a hot plate with a mechanical stirrer for a few minutes. The container was placed back in a 65° C. oven to deaerate. The molten polymer mixture was poured into an anodized aluminum metal block commercially available from Coburn, Muskogee, Okla., covered with a polyethylene film, and molded in a concave shape. The block was cooled and the polycaprolactone mixture solidified. The melting time was evaluated by observing the time in seconds that the polymer mixture took to melt at 65° C. under a 500 watt GE sun lamp held at a distance of 125 mm from the surface of the polymer.

#### Example 5

Low temperature melting plastics: candle wax, Gerber wax from Gerber Optical Inc., South Windsor, Conn., and Exxon Ethylene Vinyl Acetate (MV 02528) from Exxon Company, Houston, Tex. were each mixed with 30 weight percent carbon black commercially available as “AROSPHERE 11” from Huber Corp., Borger, Tex. The waxes and carbon black were placed in a HDPE container in an oven at 85° C. until the waxes melted. Then the container was placed in boiling water on a hot plate with a mechanical stirrer for a few minutes. The container was placed back in a 65° C. oven to deaerate. The molten polymer mixture was poured into a tray and allowed to cool and solidify. The

melting time was evaluated by observing the time in seconds that the wax mixture took to melt at 65° C. under a 500 watt GE sun lamp held at a distance of 125 mm from the surface of the polymer. Hardness was measured using ASTM D2240-91 "Shore Type 'D'".

TABLE 5a

| Run Number | Low melting Temperature Plastics (wt. %)  | Carbon Black (wt. %) | Melting Time (seconds) | Hardness ('D'/'A') |
|------------|-------------------------------------------|----------------------|------------------------|--------------------|
| 1          | ethylene vinyl acetate <sup>1</sup><br>70 | 30                   | 15                     |                    |
| 2          | candle wax<br>70                          | 30                   | 10                     |                    |
| 3          | Gerber wax <sup>2</sup><br>70             | 30                   | 5                      | 28/88              |

<sup>1</sup>"Exxon Ethylene vinyl acetate (MV 02528)" available from Exxon Chemical Company, Houston, TX

<sup>2</sup>"Gerber wax" available from Gerber Optical Inc., South Windsor, CT

Low melting plastics mixed with a heat absorbing material such as carbon black had sufficiently low melting times to be useful as a blocking material. Blending carbon black, black pigment or ceramic microspheres increased hardness. The wax used in Run 3 had a hardness of 22D before adding the carbon black.

#### Example 6

Two resins were blended on a "Haake Rheocord Extruder" (Model 252) commercially available from Haake Inc., Saddle Brook, N.J. with a 1.9 cm diameter screw and with a length to diameter (L:D) ratio of 25:1 to form the backing layer of the surface protection tape. The amounts and types of resins are listed in Table 6a. The temperature of the extruder inlet was maintained at 149° C. The extruder outlet and neck tube temperatures were kept at the same temperatures, 177° C. The die temperature was 204° C.

The deblock test was used to measure the deblocking force required to separate a blocked lens from the block. A double coated tape commercially available as "3M Double

uncut, "RLX Plus™ Scratch Resistant, Finished Lens in Hard Resin" from Signet Armorlite, Inc. using the 3M SURFACE SAVER Applicator with an air pressure setting of 0.28 MPa. Air pressure was set at 0.02–0.03 MPa for the blocker commercially available as OPTEK™ Model 200 Blocker. A brass blocking ring was placed on the blocker and a 56 mm diameter Coburn Block from Coburn Company was placed into the ring such that the inlet in the block fit snugly over the rubber nozzle. The block was centered on the lens and slowly filled with polycaprolactone from Run 1. The blocked lens assembly was allowed to set for 10 to 15 seconds after filling, in order for the resin to harden and form a good bond to the taped lens. The blocked lens was removed from the blocker and allowed to set for 1 hour before deblocking. The blocked lens was placed into the deblocking ring and the lens was taped to the deblocking ring using 1.27 cm wide filament tape. With the blocking tool facing downward, the blocked lens was placed in a hollow tube. The diameter of the tube was much greater than the blocking tool and the tube was sufficiently thick to abruptly stop the lens by its perimeter. The blocked lens assembly was dropped starting at 2.5 cm and raised in 2.5 cm increments until the block separated from the tape or until 15.2 cm in height, then, raised and dropped in 5.1 cm increments up to 91.4 cm. The height in centimeters (cm) at which the block released from the tape was recorded as the deblock values in Table 6a.

Tensile Strength and Percent Elongation in the machine and cross machine directions were determined for Runs 1–7 using ASTM Test Method D 882-91 ("Standard Test Methods for Tensile Properties of Thin Plastic Sheeting" Test Method A: Static Weighing, Constant-Rate-of-Grip Separation Test) on an "INSTRON™ Model No. 1122 Tensile Tester" from Instron Corporation, Canton, Mass. The films were tested in the machine direction and cross machine direction and the results of 3 samples in each direction were averaged. The crosshead speed was 25.4 cm/min, size of sample was 10.2 cm long, 2.54 cm wide, and 0.127 mm thick and the distance between the grips was 5.08 cm.

TABLE 6a

| Run Number | Composition                  |                 | Deblock Values (cm) | Tensile Strength        |                       | Elongation            |                     |
|------------|------------------------------|-----------------|---------------------|-------------------------|-----------------------|-----------------------|---------------------|
|            | Resin 1 <sup>1</sup> (wt. %) | Resin 2 (wt. %) |                     | Machine Direction (MPa) | Cross Direction (MPa) | Machine Direction (%) | Cross Direction (%) |
| 1          | 20                           | 80 <sup>2</sup> | 15.2                | 0.098                   | 0.066                 | 624                   | 638                 |
| 2          | 20                           | 80 <sup>3</sup> | 15.2                | 0.134                   | 0.107                 | 737                   | 799                 |
| 3          | 40                           | 60 <sup>4</sup> | 20.3                |                         |                       |                       |                     |
| 4          | 40                           | 60 <sup>2</sup> | 20.3                | 0.132                   | 0.044                 | 409                   | 457                 |
| 5          | 40                           | 60 <sup>3</sup> | 15.2                | 0.134                   | 0.046                 | 512                   | 416                 |
| 6          | 60                           | 40 <sup>2</sup> | 20.3                | 0.134                   | 0.062                 | 603                   | 446                 |
| 7          | 60                           | 40 <sup>3</sup> | 30.5                | 0.134                   | 0.069                 | 612                   | 469                 |

<sup>1</sup>"ESTANE™ 58309 Polyether Type Thermoplastic Polyurethane" from the B. F. Goodrich Company, Cleveland, OH.

<sup>2</sup>"BYNEL™ E-374 Anhydride Modified Ethylene Acrylate" from E. I. Du Pont de Nemours and Company, Wilmington, DE (now BYNEL 2174).

<sup>3</sup>"AFFINITY™ 1845 Very Low Density Polyethylene" from Dow Chemical Company, Midland, MI.

<sup>4</sup>"ASPUN™ 6806 Linear Low Density Polyethylene" from Dow Chemical Company, Midland, MI.

Coated 1512 Tape" was applied to one side of the backing layer of the lens surface protective film and to 70 mm plastic lenses with 2.0–2.4 mm center thickness, plano, finished

#### Example 7

Runs 1–3 were prepared by melt blending the amounts

and types of resins, waxes, and other additives described in Table 7a to form blocking compositions.

TABLE 7a

| Run Number | Ethylene/Vinyl Acetate <sup>1</sup><br>(parts) | Paraffin Wax <sup>2</sup><br>(parts) | Other Additives<br>(parts) |
|------------|------------------------------------------------|--------------------------------------|----------------------------|
| 1          | 200                                            | 100                                  | 15.8 <sup>3</sup>          |
| 2          | 400                                            | 200                                  | 1.2 <sup>4</sup>           |
| 3          | 100                                            | 100                                  | 0                          |

<sup>1</sup>"ELVAX™ 210" (72 weight percent ethylene/28 weight percent vinyl acetate) from E. I. Du Pont de Nemours and Company, Wilmington, DE.

<sup>2</sup>"SHELLWAX™ 200" from Shell Oil Company, Houston, TX.

<sup>3</sup>"Dow Corning 360 Silicone Medical Fluid" (20 centipoise viscosity) from Dow Corning, Midland, MI.

<sup>4</sup>"GP-1 Thixotrope" (N-lauroyl-L-glutamic acid di-n-butylamide) from Ajinomoto U.S.A., Inc., Teaneck, NJ.

In order to test the adhesion of the blocking compositions to a lens protection tape (commercially available as "SURFACE SAVER™ #1640 Lens Surface Systems" from 3M Company), a ceramic plate was clamped to the top of a laboratory bench, the lens protection tape was placed adhesive side down on the plate and a TEFLON™ Coated Mold with four 1.3 cm diameter holes was placed on top of the backing of the tape. A blend from Run 1, 2, or 3 was placed in a container on a hot plate until it was melted. Then the molten blend was poured into the holes in the mold to a depth of 0.3 to 0.6 cm. The molten blend was allowed to cool to room temperature and solidify into cylinders. The cylinders of resin/wax blend were removed from the mold. The cylinders of solidified resin/wax blend were removed from the tape by pulling them off by hand. The cylinder made in Run 1 came off the easiest and marred the tape backing the least. However, the cylinder would not come off by knocking it against the laboratory bench which is the usual method for deblocking a lens. The cylinder made in Run 2 was harder to remove than the one made in Run 1 and a little more marking was observed on the tape backing surface. The cylinder made in Run 3 was the hardest to pull off the tape backing.

In a second experiment using the same resin/wax blends, an assembly of the mold on the tape backing was clamped to a piece of acrylic film instead of the ceramic plate. Solid pieces of resin/wax blends from Runs 1, 2, or 3 were placed in the holes of the mold and the entire assembly was placed in an oven at 70° C. until the resin/wax blend had melted and flowed. The assembly was allowed to cool and the resin/wax blend solidified. The cylinders of resin/wax blends were removed from the mold and pulled off of the tape by hand. The resin/wax blend from Run 1 had very low adhesion to the backing and came off very easily. The blend from Run 2 was fairly hard to remove and left a little residue on the backing. The blend from Run 3 has hard to remove and left a lot of residue on the backing.

## Example 8

Pieces of polycaprolactone (PCL) (commercially available as "TONE™ Polyol P-300" (10,000 molecular weight) from Union Carbide Chemicals and Plastics Company Inc., Danbury, Conn.) were placed in the holes of the mold described in Example 7 and the entire assembly was placed in an oven at 70° C. until the resin had melted and flowed. The assembly was allowed to cool and the resins solidified. The cylinders of resin were removed from the mold and pulled off of the tape by hand. PCL was as hard to remove from the tape backing as the cylinders in Example 7, Runs 2 and 3. In a second experiment the lens protection tape in the assembly was replaced with an unprimed polyethylene

terephthalate (PET) film. There was no adhesion of the PCL to the PET film. In a third experiment the PET film was replaced with a polyethylene film from a "ZIPLOC™ Bag". The cylinders were very easily removed.

## Example 9

Resins were made by blending the amounts and types of resins described in Table 9a to form blocking compositions.

TABLE 9a

| Run Number | Polycaprolactone <sup>1</sup><br>(parts) | Ethylene/Vinyl Acetate<br>(parts) |
|------------|------------------------------------------|-----------------------------------|
| 1          | 400                                      | 100 <sup>2</sup>                  |
| 2          | 400                                      | 100 <sup>3</sup>                  |

<sup>1</sup>"TONE™ Polyol P-300" (10,000 molecular weight) from Union Carbide Chemicals and Plastics Company Inc.

<sup>2</sup>"ELVAX™ 210" (72 weight percent ethylene/28 weight percent vinyl acetate) (Melt Index 400) from E. I. Du Pont de Nemours and Company

<sup>3</sup>"ELVAX™ 4969-6W" (72 weight percent ethylene/28 weight percent vinyl acetate) (Melt Index 1900) from E. I. Du Pont de Nemours and Company

Pieces of the resin blends from Run 1 or Run 2 were placed in the holes of the mold described in Example 7 and the entire assembly was placed in an oven at 70° C. until the resin blends had melted and flowed. The assembly was allowed to cool and the resin blends solidified. The cylinders of resin from Run 1 or Run 2 were removed from the mold and pulled off of the tape by hand. Cylinders of resin from Run 1 were removed easily but not too easily. The viscosity of the resin blend from Run 1 was fairly high. Cylinders of resin blends from Run 2 were removed very easily and the viscosity of the resin blend from Run 2 was also fairly high.

## Example 10

A resin was made by blending 8 parts polycaprolactone (commercially available as "TONE™ Polyol P-300" (10,000 molecular weight) from Union Carbide Chemicals and Plastics Company Inc.) with 5 parts polycaprolactone (commercially available as "TONE™ Polyol 221" (1000 molecular weight) from Union Carbide Chemicals and Plastics Company Inc.). Pieces of the resin were placed in the holes of the mold described in Example 7 and the entire assembly was placed in an oven at 70° C. until the resin had melted and flowed. In this experiment the lens protection tape in the assembly was replaced with a polyethylene film from a "ZIPLOC™ Bag". The assembly was allowed to cool and the resin solidified. The cylinders were removed from the mold and pulled off of the tape by hand. The cylinders of resin were very easily removed from the film.

Melting points were determined using Differential Scanning Calorimetry (DSC) at a rate of 20° C. per minute from minus 50° C. to plus 150° C. The results are reported in Table 10a.

TABLE 10a

| Example No./Run No. | Melting Temperature<br>(°C.) |
|---------------------|------------------------------|
| 8                   | 70                           |
| 10                  | 58                           |
| 9/1                 | 61                           |
| 9/2                 | 65                           |

## Example 11

Two layer lens surface protection tapes were coextruded in a one step process. The two layers were an outer film layer and an adhesive layer.

The resins used for the film layer comprised 60 parts "ESTANE™ 58309 Polyether Type Thermoplastic Polyurethane" from the B. F. Goodrich Company; 34 parts AFFINITY™ 1845 Very Low Density Polyethylene" from Dow Chemical Company; and 6 parts "Green Pigment Number 1054" from Hoechst-Celanese Corp., Specialty Chemical Group, Coventry, R.I. The resins were blended using a 58 mm diameter twin screw extruder with a L:D ratio of 44:1 (available from Crompton & Knowles Corp., Davis Standard Division, Pawtucket, Conn.). The temperature of the extruder inlet was maintained at 38° C. and the extruder outlet and neck tube temperatures were maintained at 149° C. The target film layer caliper was 0.051 mm.

The adhesive layer was a 94 parts IOA/6 parts AA acrylic adhesive with 0.4% ABP crosslinker made by the process described in U.S. Pat. Nos. 4,737,559 and 4,847,137. The adhesive layer was processed using a 58 mm diameter twin screw extruder with a L:D ratio of 44:1 (available from Crompton & Knowles Corp.). The temperature of the extruder inlet was maintained at 93° C., the extruder outlet was at 149° C., and the neck tube temperature was maintained at 166° C. The target adhesive layer caliper was 0.076 mm.

The melt flows from the two extruders were combined into one melt stream using a "Cloeren™ Model 93-1123 feedblock" (available from The Cloeren Company, Orange, Tex.) and formed into a two layer film with the adhesive layer down using a "Cloeren EPOCH™ 3 Die" fabricated by The Cloeren Company. The feedblock and the die temperature were maintained at 177° C. The film was extruded onto a silicone release liner. The adhesive was crosslinked by irradiating the tape from the film side using UV curing lamps (available from UVEX Inc., Sunnyvale, Calif.) with a light intensity of 100 millijoules per square cm as measured by a Model M365 UV Radiometer (from Electronic Instrumentation and Technology Inc., Sterling, Va.). The target caliper for the adhesive was 0.076 mm.

The tape was evaluated for deblock force using the Deblock Test described in Example 6 except the double coated tape was not used to attach the tape to the lens surface. The average deblock value was 58.4 cm.

#### Example 12

Two layer lens surface protection tapes were coextruded in a one step process.

The resins used for the film layer comprised 56 parts "PELLETHANE™ 2103-90AE Polytetramethylene Glycol Ether Thermoplastic Polyurethane Elastomers" from Dow Chemical Company; 38 parts "ENGAGE™ 8200 Polyolefin Elastomer" from Dow Chemical Company; and 6 parts "Green Pigment Number 1054" from Hoechst-Celanese Corp. The resins were blended using the twin screw extruder described in Example 11. The temperature of the extruder inlet was maintained at 21° C. and the extruder outlet and neck tube temperatures were maintained at 166° C. The target film layer caliper was 0.051 mm.

The adhesive layer was the same as that described in Example 11. The adhesive layer was processed using the twin screw extruder described in Example 11. The temperature of the extruder inlet was maintained at 93° C., the extruder outlet was at 149° C., and the neck tube temperature varied from 177° C. to 193° C. The target adhesive layer caliper was 0.076 mm.

The melt flows from the two extruders were combined into one melt stream as described in Example 11. The feedblock temperature was maintained at 177° C. and the die

temperature was maintained at 179° C. The film was extruded onto a silicone release liner. The adhesive was crosslinked by irradiating the tape from the film side using UV curing lamps (available from UVEX Inc.) with a light intensity of 150 millijoules per square cm as measured by a Model M365 UV Radiometer (from Electronic Instrumentation and Technology Inc.). The target caliper for the adhesive was 0.076 mm.

#### Example 13

Polycaprolactone (PCL) materials available as "CAPA™ poly(ε-caprolactone) diol" (10,000 molecular weight) from Solvay Interrox, Houston, Tex., Run 1, were blended with a lower viscosity material, stearic acid (SA) available from J. T. Baker, Phillipsburg, N.J., in the amounts shown in Table 13a, Runs 2-5. The lower viscosity material, SA, was heated in an aluminum tin until liquified and allowed to cool and solidify. The PCL was heated in an aluminum tin on a hot plate to about 100° C. Chunks of SA were broken off and added slowly to the molten PCL while stirring mechanically.

TABLE 13a

| Run Number | Polycaprolactone (weight percent) | Stearic Acid (weight percent) |
|------------|-----------------------------------|-------------------------------|
| 1          | 100                               | 0                             |
| 2          | 95                                | 5                             |
| 3          | 90                                | 10                            |
| 4          | 85                                | 15                            |
| 5          | 80                                | 20                            |

Viscosity of the molten PCL/SA mixtures was determined using a Brookfield Viscometer as described in Example 3.

Hot melt blends of PCL/SA were poured into a Coburn block, then covered with polyethylene terephthalate film and allowed to solidify. Hardness was measured using a durometer for Shore type 'D' as described in Example 3 after 10, 20, and 30 minutes of cooling. The solidified PCL/SA mixture was inspected for cracking on the surface. The time required for the molten PCL/SA mixture to solidify was measured. The results of viscosity and hardness testing as well as the presence or absence of cracks and the set-up time are reported in Table 13b.

TABLE 13b

| Run Number | Viscosity (cp) | Shore "D" Hardness |        |        | Cracking (yes or no) | Set-up Time (seconds) |
|------------|----------------|--------------------|--------|--------|----------------------|-----------------------|
|            |                | 10 min             | 20 min | 30 min |                      |                       |
| 1          | 30,000         | 37                 | 41     | 44     | no                   | >30                   |
| 2          | 18,000         | 37                 | 39     | 38     | no                   | 10-15                 |
| 3          | 14,400         | 27                 | 30     | 36     | no                   | —                     |
| 4          | 10,600         | 24                 | 28     | 34     | no                   | —                     |
| 5          | 8,300          | 20                 | 27     | 30     | no                   | —                     |

The viscosity of PCL was decreased by a factor of about 4 when 20 percent SA was added to the melt.

#### Example 14

Polycaprolactone (PCL) materials available as "CAPA™ poly(ε-caprolactone) diol" (10,000 molecular weight) from Solvay Interrox, Houston, Tex., were blended with a lower viscosity material, stearyl alcohol (SAL) or 1-octadecanol available from Aldrich Chemical Company, Milwaukee, Wis., as described in Example 13 in the amounts shown in Table 14a.

TABLE 14a

| Run Number | Polycaprolactone (weight percent) | Stearyl alcohol (weight percent) |
|------------|-----------------------------------|----------------------------------|
| 1          | 100                               | 0                                |
| 2          | 95                                | 5                                |
| 3          | 90                                | 10                               |
| 4          | 85                                | 15                               |
| 5          | 80                                | 20                               |

The blocking compositions of molten PCL/SAL blends were evaluated for viscosity, hardness, and cracking, as described for Example 13. The results are reported in Table 14b.

TABLE 14b

| Run Number | Viscosity (cp) | Shore "D" Hardness |        |        | Cracking (yes or no) |
|------------|----------------|--------------------|--------|--------|----------------------|
|            |                | 10 min             | 20 min | 30 min |                      |
| 1          | 30,000         | 37                 | 41     | 44     | no                   |
| 2          | 16,600         | 35                 | 39     | 43     | no                   |
| 3          | 12,200         | 24                 | 29     | 31     | no                   |
| 4          | 8,920          | 19                 | 24     | 28     | no                   |
| 5          | 6,720          | 18                 | 24     | 27     | no                   |

SAL is less acidic than SA.

Example 15

Polycaprolactone (PCL) materials available as "CAPA™ poly( $\epsilon$ -caprolactone) diol" (10,000 molecular weight) from Solvay Interrox, Houston, Tex., were blended with lower viscosity materials, stearic acid (SA) and stearyl alcohol (SAL). Chunks of solidified, blended SA and SAL in a ratio of 64 parts by weight SA to 36 parts by weight SAL were added to the molten PCL as described in Example 13 in the amounts shown in Table 15a.

TABLE 15a

| Run Number | Polycaprolactone (weight percent) | Stearic Acid: Stearyl alcohol (weight percent) |
|------------|-----------------------------------|------------------------------------------------|
| 1          | 100                               | 0                                              |
| 2          | 95                                | 5                                              |
| 3          | 90                                | 10                                             |
| 4          | 85                                | 15                                             |
| 5          | 80                                | 20                                             |

The blocking compositions of molten PCL/SAL blends were evaluated for viscosity, hardness, and cracking, as described for Example 13. The results are reported in Table 15b.

TABLE 15b

| Run Number | Viscosity (cp) | Shore "D" Hardness |        |        | Cracking (yes or no) |
|------------|----------------|--------------------|--------|--------|----------------------|
|            |                | 10 min             | 20 min | 30 min |                      |
| 1          | 30,000         | 37                 | 41     | 44     | no                   |
| 2          | 17,900         | 34                 | 41     | 41     | no                   |
| 3          | 12,400         | 32                 | 35     | 36     | no                   |
| 4          | 8,000          | 28                 | 32     | 32     | no                   |
| 5          | 5,500          | 27                 | 31     | 31     | no                   |

The blend solidified faster than PCL alone.

Example 16

5 Polycaprolactone (PCL) materials available as "TONE™ P-300 polycaprolactone" (10,000 molecular weight) from Union Carbide Corporation, Danbury, Conn. were blended with a lower viscosity material, tri-phenyl phosphate (TPP) available from Monsanto Chemical Company, St. Louis, Mo., as described in Example 13 in the amounts shown in Table 16a.

TABLE 16a

| Run Number | Polycaprolactone (weight percent) | Tri-phenyl phosphate (weight percent) |
|------------|-----------------------------------|---------------------------------------|
| 1          | 100                               | 0                                     |
| 2          | 95                                | 5                                     |
| 3          | 90                                | 10                                    |
| 4          | 85                                | 15                                    |

20 The blocking compositions of molten PCL/TPP blends were evaluated for viscosity, hardness, and cracking as described for Example 13. The results are reported in Table 16b.

TABLE 16b

| Run Number | Viscosity (cp) | Shore "D" Hardness |        |        | Cracking (yes or no) |
|------------|----------------|--------------------|--------|--------|----------------------|
|            |                | 10 min             | 20 min | 30 min |                      |
| 1          | 54,000         | 37                 | 41     | 44     | no                   |
| 2          | 44,200         | 38                 | 40     | 41     | no                   |
| 3          | 35,500         | 34                 | 35     | 36     | no                   |
| 4          | 30,000         | 30                 | 31     | 31     | no                   |

35 The viscosity of PCL was decreased by a factor of about 2 when 15 percent TPP was added to the melt.

Example 17

40 Polycaprolactone materials available as "CAPA™ poly( $\epsilon$ -caprolactone) diol" (10,000 molecular weight) from Solvay Interrox, Houston, Tex., were blended with a lower viscosity material, myristyl alcohol (MAL) (1-tetradecanol) available from Aldrich Chemical Company as described in Example 13 in the amounts shown in Table 17a.

TABLE 17a

| Run Number | Polycaprolactone (weight percent) | Myristyl alcohol (weight percent) |
|------------|-----------------------------------|-----------------------------------|
| 1          | 100                               | 0                                 |
| 2          | 95                                | 5                                 |
| 3          | 90                                | 10                                |
| 4          | 85                                | 15                                |
| 5          | 70                                | 30                                |

50 The blocking compositions of molten PCL/MAL blends were evaluated for viscosity as described for Example 3 except spindle no. 16 was used. The molten blends were poured into a mold, allowed to cool and solidify, and evaluated for Tangent Modulus of Elasticity in Bending and Flexural Strength as described for Example 2 except the crosshead motion was 2.8 mm per minute. The results are reported in Tables 17b and 17c.

TABLE 17b

| Tangent Modulus of Elasticity in Bending |                   |            |                          |
|------------------------------------------|-------------------|------------|--------------------------|
| Run Number                               | Number of Samples | Mean (MPa) | Standard Deviation (MPa) |
| 5                                        | 5                 | 434        | 19                       |

TABLE 17c

| Flexural Strength |                   |            |                          |
|-------------------|-------------------|------------|--------------------------|
| Run Number        | Number of Samples | Mean (MPa) | Standard Deviation (MPa) |
| 5                 | 5                 | 3.3        | 0.3                      |

Example 18

Polycaprolactone materials available as "CAPA™ poly (ε-caprolactone) diol" (10,000 molecular weight) from Solvay Interrox, Houston, Tex. were blended with lower viscosity materials, myristyl alcohol (MAL) (1-tetradecanol) and stearyl alcohol (SAL) (1-octadecanol) available from Aldrich Chemical Company. Chunks of blended and solidified MAL and SAL were added as described in Example 13 in the amounts shown in Table 18a.

TABLE 18a

| Run Number | Polycaprolactone (weight percent) | Myristyl alcohol (weight percent) | Stearyl alcohol (weight percent) |
|------------|-----------------------------------|-----------------------------------|----------------------------------|
| 1          | 80                                | 6                                 | 14                               |
| 2          | 80                                | 7                                 | 13                               |
| 3          | 80                                | 8                                 | 12                               |
| 4          | 80                                | 9                                 | 11                               |

The blocking compositions of molten PCL/MAL/SAL blends were evaluated for viscosity as described for Example 3, except spindle no. 16 was used. The molten blends were poured into a mold, allowed to cool and solidify, and evaluated for Tangent Modulus of Elasticity in Bending and Flexural Strength as described for Example 2 except the crosshead motion was 2.8 mm per minute. The results are reported in Tables 18b and 18c.

TABLE 18b

| Tangent Modulus of Elasticity in Bending |                |                   |            |                          |
|------------------------------------------|----------------|-------------------|------------|--------------------------|
| Run Number                               | Viscosity (cp) | Number of Samples | Mean (MPa) | Standard Deviation (MPa) |
| 1                                        | 6,000          | 5                 | 436        | 31                       |
| 2                                        | 6,000          | 5                 | 506        | 29                       |
| 3                                        | 5,900          | 5                 | 454        | 34                       |
| 4                                        | 5,800          | 5                 | 471        | 39                       |

TABLE 18c

| Flexural Strength |                   |            |                          |
|-------------------|-------------------|------------|--------------------------|
| Run Number        | Number of Samples | Mean (MPa) | Standard Deviation (MPa) |
| 1                 | 5                 | 3.2        | 0.4                      |
| 2                 | 5                 | 3.2        | 0.3                      |

TABLE 18c-continued

| Flexural Strength |                   |            |                          |
|-------------------|-------------------|------------|--------------------------|
| Run Number        | Number of Samples | Mean (MPa) | Standard Deviation (MPa) |
| 3                 | 5                 | 3.3        | 0.2                      |
| 4                 | 5                 | 3.5        | 0.3                      |

Example 19

Polycaprolactone materials available as "CAPA™ poly (ε-caprolactone) diol" (10,000 molecular weight) from Solvay Interrox, Houston, Tex. were blended with lower viscosity materials, dodecyl alcohol (DO) (1-octadecanol) available from Eastman Chemical Company, Kingsport, Tenn., myristyl alcohol (MAL) (1-tetradecanol) and stearyl alcohol (SAL) (1-octadecanol) available from Aldrich Chemical Company. Chunks of blended and solidified DO, MAL, and SAL were added as described in Example 13 in the amounts shown in Table 19a.

TABLE 19a

| Run Number | Polycaprolactone (weight percent) | Dodecyl alcohol (weight percent) | Myristyl alcohol (weight percent) | Stearyl alcohol (weight percent) |
|------------|-----------------------------------|----------------------------------|-----------------------------------|----------------------------------|
| 1          | 95                                | 0.1                              | 1.7                               | 3.2                              |
| 2          | 90                                | 0.2                              | 3.4                               | 6.4                              |
| 3          | 85                                | 0.3                              | 5.1                               | 9.6                              |
| 4          | 80                                | 0.4                              | 6.8                               | 12.8                             |

The blocking compositions of molten PCL/DO/MAL/SAL blends were evaluated for viscosity as described for Example 3 except spindle no. 16 was used. The molten blends were poured into a mold, allowed to cool and solidify, and evaluated for Tangent Modulus of Elasticity in Bending and Flexural Strength as described for Example 2 except the crosshead motion was 2.8 mm per minute. The results are reported in Tables 19b and 19c.

TABLE 19b

| Tangent Modulus of Elasticity in Bending |                |                   |            |                          |
|------------------------------------------|----------------|-------------------|------------|--------------------------|
| Run Number                               | Viscosity (cp) | Number of Samples | Mean (MPa) | Standard Deviation (MPa) |
| 1                                        | 16,400         | 5                 | 566        | 49                       |
| 2                                        | 11,600         | 5                 | 521        | 15                       |
| 3                                        | 7,800          | 5                 | 447        | 42                       |
| 4                                        | 5,600          | 5                 | 509        | 30                       |

TABLE 19c

| Flexural Strength |                   |            |                          |
|-------------------|-------------------|------------|--------------------------|
| Run Number        | Number of Samples | Mean (MPa) | Standard Deviation (MPa) |
| 1                 | 5                 | 1.9        | 0.03                     |
| 2                 | 5                 | 2.3        | 0.2                      |
| 3                 | 5                 | 2.3        | 0.1                      |
| 4                 | 5                 | 3.2        | 0.2                      |

Example 20

Polycaprolactone materials available as "CAPA™ poly (ε-caprolactone) diol" (10,000 molecular weight) from

Solvay Interox, Houston, Tex. were blended with polyethylene glycol methyl ether (2,000 molecular weight) (PEGME) available from Aldrich Chemical Company as described in Example 13 in the amounts shown in Table 20a.

TABLE 20a

| Run Number | Polycaprolactone (weight percent) | Polyethylene glycol methyl ether (weight percent) |
|------------|-----------------------------------|---------------------------------------------------|
| 1          | 90                                | 10                                                |
| 2          | 80                                | 20                                                |
| 3          | 70                                | 30                                                |

The molten PCL/PEGMA blends were poured into a mold, allowed to cool and solidify, and evaluated for Tangent Modulus of Elasticity in Bending and Flexural Strength as described for Example 2 except the crosshead motion was 2.8 mm per minute. The results are reported in Tables 20b and 20c.

TABLE 20b

| Tangent Modulus of Elasticity in Bending |                   |            |                          |
|------------------------------------------|-------------------|------------|--------------------------|
| Run Number                               | Number of Samples | Mean (MPa) | Standard Deviation (MPa) |
| 1                                        | 5                 | 491        | 34                       |
| 2                                        | 5                 | 478        | 30                       |
| 3                                        | 5                 | 589        | 27                       |

TABLE 20c

| Flexural Strength |                   |            |                          |
|-------------------|-------------------|------------|--------------------------|
| Run Number        | Number of Samples | Mean (MPa) | Standard Deviation (MPa) |
| 1                 | 5                 | 2.6        | 0.2                      |
| 2                 | 5                 | 3.5        | 0.3                      |
| 3                 | 5                 | 3.2        | 0.4                      |

## Example 21

Polycaprolactone materials available as "CAPA™ poly (ε-caprolactone) diol" (8,000 molecular weight), "CAPA™ poly(ε-caprolactone) diol" (10,000 molecular weight), and "CAPA™ poly(ε-caprolactone) diol" (12,000 molecular weight) from Solvay Interox were blended with polyethylene glycol (1500 or 2000 molecular weight (MW)) (PEG) available from Aldrich Chemical Company as described in Example 13 in the amounts shown in Table 21a.

TABLE 21a

| Run Number | Polycaprolactone (weight percent) |                      |                      | Polyethylene ethylene glycol (weight percent) |         |
|------------|-----------------------------------|----------------------|----------------------|-----------------------------------------------|---------|
| Number     | "P-8K" <sup>1</sup>               | "P-10K" <sup>2</sup> | "P-12K" <sup>3</sup> | 1500 MW                                       | 2000 MW |
| 1          | —                                 | 90                   | —                    | 10                                            | —       |
| 2          | —                                 | 80                   | —                    | 20                                            | —       |
| 3          | 90                                | —                    | —                    | —                                             | 10      |
| 4          | 80                                | —                    | —                    | —                                             | 20      |

TABLE 21a-continued

| Run Number | Polycaprolactone (weight percent) |                      |                      | Polyethylene ethylene glycol (weight percent) |         |
|------------|-----------------------------------|----------------------|----------------------|-----------------------------------------------|---------|
|            | "P-8K" <sup>1</sup>               | "P-10K" <sup>2</sup> | "P-12K" <sup>3</sup> | 1500 MW                                       | 2000 MW |
| 5          | 5                                 | —                    | 90                   | —                                             | 10      |
| 6          | —                                 | —                    | —                    | 90                                            | —       |

1 "CAPA™ poly(ε-caprolactone diol)" (8,000 molecular weight) from Solvay Interox, Houston, TX.

2 "CAPA™ poly(ε-caprolactone diol)" (10,000 molecular weight) from Solvay Interox.

3 "CAPA™ poly(ε-caprolactone diol)" (12,000 molecular weight) from Solvay Interox.

15

The blocking compositions of molten PCL/PEG blends were evaluated for viscosity as described for Example 3 except spindle no. 16 was used. The molten blends were poured into a mold, allowed to cool and solidify, and evaluated for Tangent Modulus of Elasticity in Bending and Flexural Strength as described for Example 2 except the crosshead motion was 2.8 mm per minute. The results are reported in Tables 21b and 21c.

TABLE 21b

| Tangent Modulus of Elasticity in Bending |                |                   |            |                          |
|------------------------------------------|----------------|-------------------|------------|--------------------------|
| Run Number                               | Viscosity (cp) | Number of Samples | Mean (MPa) | Standard Deviation (MPa) |
| 1                                        | 17,000         | 5                 | 419        | 22                       |
| 2                                        | 11,000         | 5                 | 404        | 35                       |
| 3                                        | 8,300          | 5                 | 493        | 17                       |
| 4                                        | 6,200          | 5                 | 430        | 64                       |
| 5                                        | 16,200         | 5                 | 525        | 42                       |
| 6                                        | 31,000         | 4                 | 454        | 34                       |

TABLE 21c

| Flexural Strength |                   |            |                          |
|-------------------|-------------------|------------|--------------------------|
| Run Number        | Number of Samples | Mean (MPa) | Standard Deviation (MPa) |
| 1                 | 5                 | 3.4        | 0.5                      |
| 2                 | 5                 | 2.1        | 0.7                      |
| 3                 | 5                 | 2.4        | 0.3                      |
| 4                 | 5                 | 4.2        | 0.9                      |
| 5                 | 5                 | 2.0        | 0.3                      |
| 6                 | 4                 | 3.0        | 0.5                      |

Example 22

High molecular weight polycaprolactone materials available as "CAPA™ 630" (30,000 molecular weight) from Solvay Interox were blended with lower viscosity materials, a low molecular weight polycaprolactone available as "TONE™ P-1270" (4,000 molecular weight) from Union Carbide Chemicals and Plastics Company Inc. polycaprolactone (PCL) and, myristyl alcohol (MAL) (1-tetradecanol) available from Aldrich Chemical Company. Chunks of a low molecular weight PCL and MAL were added as described in Example 13 in the amounts shown in Table 22a.

TABLE 22a

| Run    | Polycaprolactone<br>(weight percent) |                             | Myristyl alcohol |
|--------|--------------------------------------|-----------------------------|------------------|
| Number | "CAPA™ 630" <sup>1</sup>             | "TONE™ P-1270" <sup>2</sup> | (weight percent) |
| 1      | 44                                   | 20                          | 36               |
| 2      | 43                                   | 36                          | 21               |

<sup>1</sup>Commercially available from Solvay Interox, Houston, TX.

<sup>2</sup>Commercially available from Union Carbide Chemicals and Plastics Company Inc., Danbury, CT.

The blocking compositions of molten PCL/MAL blends were evaluated for viscosity as described for Example 3 except spindle no. 16 was used. The molten blends were poured into a mold, allowed to cool and solidify, and evaluated for Tangent Modulus of Elasticity in Bending and Flexural Strength as described for Example 2 except the crosshead motion was 2.8 mm per minute. The results are reported in Tables 22b and 22c.

TABLE 22b

| Tangent Modulus of Elasticity in Bending |                |                   |            |                          |
|------------------------------------------|----------------|-------------------|------------|--------------------------|
| Run Number                               | Viscosity (cp) | Number of Samples | Mean (MPa) | Standard Deviation (MPa) |
| 1                                        | 22,000         | 5                 | 336        | 23                       |
| 2                                        | 22,000         | 5                 | 396        | 24                       |

TABLE 22c

| Flexural Strength |                   |            |                    |
|-------------------|-------------------|------------|--------------------|
| Run Number        | Number of Samples | Mean (MPa) | Standard Deviation |
| 1                 | 5                 | 5.0        | 0.7                |
| 2                 | 5                 | 4.4        | 0.4                |

Example 23

High molecular weight polycaprolactone materials available as "CAPA™ 630" (30,000 molecular weight) from Solvay Interox were blended with lower viscosity materials, a low molecular weight polycaprolactone available as "TONE™ P-1270" from Union Carbide Chemicals and Plastics Company Inc. polycaprolactone (PCL), myristyl alcohol (MAL) (1-tetradecanol) and stearyl alcohol (SAL) (1-octadecanol) available from Aldrich Chemical Company. Chunks of blended and solidified low molecular weight PCL, MAL, and SAL were added as described in Example 13 in the amounts shown in Table 23a.

TABLE 23a

| Run Number | Polycaprolactone<br>(weight percent) |                             | Myristyl alcohol<br>(weight percent) | Stearyl alcohol<br>(weight percent) |
|------------|--------------------------------------|-----------------------------|--------------------------------------|-------------------------------------|
| Run Number | "CAPA™ 630" <sup>1</sup>             | "TONE™ P-1270" <sup>2</sup> |                                      |                                     |
| 1          | 41                                   | 30                          | 20                                   | 10                                  |

<sup>1</sup>Commercially available from Solvay Interox, Houston, TX.

<sup>2</sup>Commercially available from Union Carbide Chemicals and Plastics Company Inc., Danbury, CT.

The blocking compositions of molten PCL/MAL/SAL blends were evaluated for viscosity as described for

Example 3 except spindle no. 16 was used. The molten blends were poured into a mold, allowed to cool and solidify, and evaluated for Tangent Modulus of Elasticity in Bending and Flexural Strength as described for Example 2 except the crosshead motion was 2.8 mm per minute. The results are reported in Tables 23b and 23c.

TABLE 23b

| Tangent Modulus of Elasticity in Bending |                |                   |            |                          |
|------------------------------------------|----------------|-------------------|------------|--------------------------|
| Run Number                               | Viscosity (cp) | Number of Samples | Mean (MPa) | Standard Deviation (MPa) |
| 1                                        | 21,000         | 5                 | 303        | 66                       |

TABLE 23c

| Flexural Strength |                   |            |                          |
|-------------------|-------------------|------------|--------------------------|
| Run Number        | Number of Samples | Mean (MPa) | Standard Deviation (MPa) |
| 1                 | 5                 | 4.6        | 0.6                      |

Example 24

High molecular weight polycaprolactone materials available as "CAPA™ 630" (30,000 molecular weight) from Solvay Interox were blended with lower viscosity materials, a low molecular weight polycaprolactone material available as "TONE™ P-1270" (4,000 molecular weight) from Union Carbide Chemicals and Plastics Company Inc. polycaprolactone (PCL), myristyl alcohol (MAL) (1-tetradecanol), stearyl alcohol (SAL) (1-octadecanol) and polyethylene glycol (PEG) available from Aldrich Chemical Company. Chunks of blended and solidified low molecular weight PCL, MAL, Sal, and PEG were added as described in Example 13 in the amounts shown in Table 24a.

TABLE 24a

| Run Number | Polycaprolactone<br>(weight percent) |                             | Myristyl alcohol<br>(weight percent) | Stearyl alcohol<br>(weight percent) | Polyethylene Glycol<br>(weight percent) |
|------------|--------------------------------------|-----------------------------|--------------------------------------|-------------------------------------|-----------------------------------------|
|            | "CAPA™ 630" <sup>1</sup>             | "TONE™ P-1270" <sup>2</sup> |                                      |                                     |                                         |
| 1          | 43                                   | 20                          | 19                                   | 9                                   | 9                                       |
| 2          | 41                                   | 24                          | 16                                   | 9                                   | 11                                      |
| 3          | 42                                   | 24                          | 15                                   | 5                                   | 15                                      |
| 4          | 42                                   | 18                          | 18                                   | 10                                  | 12                                      |

<sup>1</sup>Commercially available from Solvay Interox, Houston, TX.

<sup>2</sup>Commercially available from Union Carbide Chemicals and Plastics Company Inc., Danbury, CT.

The blocking compositions of molten PCL/MAL/SAL/PEG blends were evaluated for viscosity as described for Example 3 except spindle no. 16 was used. The molten blends were poured into a mold, allowed to cool and solidify, and evaluated for Tangent Modulus of Elasticity in Bending and Flexural Strength as described for Example 2 except the crosshead motion was 2.8 mm per minute. The results are reported in Tables 24b and 24c.

TABLE 24b

| Tangent Modulus of Elasticity in Bending |                |                   |            |                          |
|------------------------------------------|----------------|-------------------|------------|--------------------------|
| Run Number                               | Viscosity (cp) | Number of Samples | Mean (MPa) | Standard Deviation (MPa) |
| 1                                        | 18,000         | 5                 | 319        | 24                       |
| 2                                        | 13,000         | 5                 | 255        | 26                       |
| 3                                        | 14,000         | 3                 | 290        | 5                        |
| 4                                        | 17,000         | 5                 | 316        | 35                       |

TABLE 24c

| Flexural Strength |                   |            |                          |
|-------------------|-------------------|------------|--------------------------|
| Run Number        | Number of Samples | Mean (MPa) | Standard Deviation (MPa) |
| 1                 | 5                 | 3.6        | 0.6                      |
| 2                 | 5                 | 4.3        | 0.3                      |
| 3                 | 3                 | 4.4        | 0.1                      |
| 4                 | 5                 | 3.7        | 0.6                      |

## Example 25

Three layer lens surface protection tapes were coextruded in a one step process. The three layers were an outer film layer (skin), a tie layer (core) and an adhesive layer. The compositions of the various layers used to make the tapes are given in Table 25a. The target thickness for the outer film layer, tie layer, and adhesive layer are reported in Table 25b.

The outer film layer was either a blend of polycaprolactone (PCL) (available as "CAPA™ 650" from Solvay Interrox) and a maleic anhydride modified ethylene acrylate (available as "Bynel 2174" from DuPont Packaging & Industrial Polymers, Wilmington, Del.) and a maleic anhydride modified linear low density polyethylene (available as "Bynel 4109" from DuPont Packaging & Industrial Polymers) or a blend of the PCL and a maleic anhydride modified low density polyethylene (available as "Bynel 4206" from DuPont Packaging & Industrial Polymers). Three percent of a pigment (available as "05ELD-1054"

from Resco Colours a division of Hoechst, Mississauga, Ontario) was added to this blend. The resins and pigment as described in Table 25a were blended using a 58 mm diameter twin screw extruder with a length to diameter (L:D) ratio of 44:1 (available from Crompton & Knowles Corp., Davis Standard Division). The temperature of the extruder inlet was maintained at 21° C. and the extruder outlet and neck tube temperatures were maintained at 193° C.

The tie layer was made from a nylon 6/6,9 copolymer (available as "GRILON™ CF62BSE Nylon 6/6,9 Copolymer" from EMS-American Grilon Inc., Sumter, S.C.). The tie layer (core) was processed using a 6.35 cm (2.5 inch) diameter single screw extruder with a length to diameter (L:D) ratio of 30:1 (available from Crompton & Knowles Corp., Davis Standard Division). The temperature of the extruder inlet was maintained at 66° C. and the extruder outlet and neck tube temperatures were maintained at 177° C.

The adhesive layer was made from a 94 parts IOA/6 parts AA acrylic adhesive with 0.4% ABP crosslinker made by the process described in U.S. Pat. Nos. 4,737,559 and 4,847,137. The adhesive layer was processed using a 58 mm diameter twin screw extruder with a length to diameter (L:D) ratio of 44:1 (available from Crompton & Knowles Corp., Davis Standard Division). The temperature of the extruder inlet was maintained at 93° C. and the extruder outlet and neck tube temperatures were maintained at 177° C.

The melt streams from the three extruders were combined into one melt stream using a "Cloeren™ Model 92-1033 feedblock" (available from The Cloeren Company) and formed into a film using a Cloeren Epoch die fabricated by The Cloeren Company. The feedblock temperature was maintained at 177° C. and the die temperature was maintained at 179° C.

The adhesive was crosslinked by irradiating the tape from the adhesive side using UV curing lamps (available from UVEK Inc., Sunnyvale, Calif.) with a light intensity of 84 millijoules/square cm as measured by a Model M365 UV Radiometer (from Electronic Instrumentation and Technology Inc., Sterling, Va.) in the 320 to 390 nm range.

TABLE 25a

| Run Number | Composition                  |                              |                              |                              |                              |                                     |
|------------|------------------------------|------------------------------|------------------------------|------------------------------|------------------------------|-------------------------------------|
|            | Film Layer <sup>1</sup>      |                              |                              |                              | Tie Layer                    |                                     |
|            | Resin 1 <sup>2</sup> (wt. %) | Resin 2 <sup>3</sup> (wt. %) | Resin 3 <sup>4</sup> (wt. %) | Resin 4 <sup>5</sup> (wt. %) | Resin 6 <sup>6</sup> (wt. %) | Adhesive Layer <sup>7</sup> (wt. %) |
| 1          | 10                           | 87                           | —                            | —                            | 100                          | 100                                 |
| 2          | 20                           | 77                           | —                            | —                            | 100                          | 100                                 |
| 3          | 30                           | 67                           | —                            | —                            | 100                          | 100                                 |
| 4          | 40                           | 57                           | —                            | —                            | 100                          | 100                                 |
| 5          | 50                           | 47                           | —                            | —                            | 100                          | 100                                 |
| 6          | 30                           | —                            | 47                           | 23                           | 100                          | 100                                 |
| 7          | 40                           | —                            | 37                           | 23                           | 100                          | 100                                 |

<sup>1</sup>The Film Layer of Runs 1-5 also contain 3 weight percent pigment, commercially available as "05ELD-1054" from Resco Colours a Division of Hoechst, Mississauga, Ontario.

<sup>2</sup>Commercially available as "CAPA™ 650 polycaprolactone" from Solvay Interrox, Houston, TX.

<sup>3</sup>Commercially available as "Bynel 4206 maleic anhydride modified low density polyethylene" from DuPont Packaging & Industrial Polymers, Wilmington, DE.

<sup>4</sup>Commercially available as "Bynel 2174 maleic anhydride modified ethylene acrylate" from DuPont Packaging & Industrial Polymers.

<sup>5</sup>Commercially available as "Bynel 4109 maleic anhydride modified linear low density polyethylene" from DuPont Packaging & Industrial Polymers.

TABLE 25a-continued

| Run Number                      | Composition                     |                                 |                                 |                                 |                       |                |
|---------------------------------|---------------------------------|---------------------------------|---------------------------------|---------------------------------|-----------------------|----------------|
|                                 | Film Layer <sup>1</sup>         |                                 |                                 | Tie Layer                       |                       | Adhesive Layer |
| Resin 1 <sup>2</sup><br>(wt. %) | Resin 2 <sup>3</sup><br>(wt. %) | Resin 3 <sup>4</sup><br>(wt. %) | Resin 4 <sup>5</sup><br>(wt. %) | Resin 6 <sup>6</sup><br>(wt. %) | Adhesive 7<br>(wt. %) |                |
|                                 |                                 |                                 |                                 |                                 |                       |                |

<sup>6</sup>Commercially available as "GRILON™ CF62BSE Nylon 6/6,9 Copolymer" from EMS-American Grilon Inc., Sumter, SC.

<sup>7</sup>94 parts IOA/6 parts AA with 0.4% ABP crosslinker, made by the process described in U.S. Pat. Nos. 4,737,559 and 4,847,137.

The lens surface protection tapes were evaluated using the Deblock Test described in Example 6 except that a second set of blocked lens were deblocked after being allowed to set for 17 hours. The results are reported in Table 25b.

TABLE 25b

| Run Number | Target Thickness      |                |                     |                       |               |  |
|------------|-----------------------|----------------|---------------------|-----------------------|---------------|--|
|            | Outer Film Layer (mm) | Tie Layer (mm) | Adhesive Layer (mm) | Deblock Values after: |               |  |
|            |                       |                |                     | 1 hour (cm)           | 17 hours (cm) |  |
| 1          | 0.0508                | 0.0076         | 0.0762              | 8.4                   | 10.9          |  |
| 2          | 0.0508                | 0.0076         | 0.0762              | na <sup>1</sup>       | na            |  |
| 3          | 0.0508                | 0.0076         | 0.0762              | 10.2                  | 13.5          |  |
| 4          | 0.0508                | 0.0076         | 0.0762              | na                    | na            |  |
| 5          | 0.0508                | 0.0076         | 0.0762              | 32.0                  | 32.3          |  |
| 6          | 0.0508                | 0.0076         | 0.0762              | 18.5                  | 18.5          |  |
| 7          | 0.0508                | 0.0076         | 0.0762              | 23.6                  | 25.4          |  |

<sup>1</sup>"na" means not available.

Example 26

Side chain crystallizable hydrocarbon polymer materials available as "VYBAR" 103 and "VYBAR" 253 from Petro-  
lite Corporation, Tulsa, Okla., were blended with a hydro-  
carbon resin available as "REGALITE" R-91, from  
Hercules, Wilmington, Del. The materials were added in  
solid form to an aluminum tin and heated until molten and  
stirred in the amounts shown in Table 26a.

The blocking compositions of molten "VYBAR"/  
"REGALITE" blends were evaluated for viscosity as  
described in Example 3 except spindle no. 16 was used and  
the temperature was 70° C. The molten blends were poured  
into a silicon elastomer mold, allowed to cool and solidify,  
and evaluated for Tangent Modulus of Elasticity in Bending  
and Flexural Strength as described in Example 2 except the  
crosshead motion was 1.27 mm per minute and the sample  
size was approximately 125 mm long, 12.7 mm wide, and  
3.18 mm thick. The span tested was 50.8 mm long giving a  
span to depth ratio equal to about 16:1. In some cases the  
material did not break at outer fiber strains up to 5%. In these  
cases the Flexural Yield Strength was calculated by using the  
point on the load-deflection curve at which the load did not  
increase with an increase in deflection. The results are  
reported in Tables 26b and 26c.

15

TABLE 26a

| Run Number | Hydrocarbon Polymer 1 <sup>1</sup><br>(weight percent) | Hydrocarbon Polymer 2 <sup>2</sup><br>(weight percent) | Hydrocarbon Resin 1 <sup>3</sup><br>(weight percent) |
|------------|--------------------------------------------------------|--------------------------------------------------------|------------------------------------------------------|
| 1          | 18.4                                                   | 18.4                                                   | 63.2                                                 |
| 2          | 40.0                                                   | 30.0                                                   | 30.0                                                 |

<sup>1</sup>Commercially available as VYBAR™ 103 from Petrolite, Tulsa, OK.

<sup>2</sup>Commercially available as VYBAR™ 253 from Petrolite, Tulsa, OK.

<sup>3</sup>Commercially available as REGALITE™ R-91 from Hercules, Inc.,  
Wilmington, DE.

20

TABLE 26b

| Number | Tangent Modulus of Elasticity in Bending<br>(ASTM D790-86) |                   |            |                          |
|--------|------------------------------------------------------------|-------------------|------------|--------------------------|
|        | Viscosity (cp)                                             | Number of Samples | Mean (MPa) | Standard Deviation (MPa) |
| 1      | 1454                                                       | 5                 | 63.6       | 17.2                     |
| 2      | 324                                                        | 5                 | 70.3       | 4.6                      |

25

TABLE 26c

| Run Number | Flexural Strength (ASTM D790-86) |                  |                          |
|------------|----------------------------------|------------------|--------------------------|
|            | Number of Samples                | Mean (MPa)       | Standard Deviation (MPa) |
| 1          | 5                                | 1.6 <sup>1</sup> | 0.2                      |
| 2          | 5                                | 2.2              | 0.2                      |

<sup>1</sup>Flexural Yield Strength

30

Example 27

Side chain crystallizable hydrocarbon polymer materials available as "VYBAR" 103 and "VYBAR" 253 from Petro-  
lite Corporation, Tulsa, Okla., were blended with a hydro-  
carbon resin available as "REGALITE" R-91, from  
Hercules, Wilmington, Del. Various levels of stearyl alcohol  
and myristyl alcohol were added to the mixture. The materials  
were added in solid form to an aluminum tin and heated until  
molten and stirred in the amounts shown in Table 27a.

35

The blocking compositions of molten "VYBAR"/  
"REGALITE"/fatty alcohol blends were evaluated for vis-  
cosity as described in Example 3 except spindle no. 16 was  
used and the temperature was 70° C. The molten blends were  
poured into a mold, allowed to cool and solidify, and  
evaluated for Tangent Modulus of Elasticity in Bending and  
Flexural Strength as described in Example 26. The results  
are reported in Tables 27b and 27c.

TABLE 27a

| Run Number | Hydrocarbon Polymer 1 <sup>1</sup><br>(weight percent) | Hydrocarbon Polymer 2 <sup>2</sup><br>(weight percent) | Hydrocarbon Resin 1 <sup>3</sup><br>(weight percent) | Stearyl Alcohol<br>(weight percent) | Myristyl Alcohol<br>(weight percent) |
|------------|--------------------------------------------------------|--------------------------------------------------------|------------------------------------------------------|-------------------------------------|--------------------------------------|
| 1          | 17.5                                                   | 17.5                                                   | 60                                                   | 2.5                                 | 2.5                                  |
| 2          | 17.5                                                   | 17.5                                                   | 50                                                   | 15.0                                | 0.0                                  |
| 3          | 17.5                                                   | 17.5                                                   | 50                                                   | 0.0                                 | 15.0                                 |
| 4          | 40                                                     | 7.5                                                    | 50                                                   | 0.0                                 | 2.5                                  |
| 5          | 19.4                                                   | 34.4                                                   | 45                                                   | 0.0                                 | 1.2                                  |
| 6          | 14.5                                                   | 14.5                                                   | 65                                                   | 3.0                                 | 3.0                                  |

<sup>1</sup>Commercially available as VYBAR™ 103 from Petrolite, Tulsa, OK.<sup>2</sup>Commercially available as VYBAR™ 253 from Petrolite, Tulsa, OK.<sup>3</sup>Commercially available as REGALITE™ R-91 from Hercules, Inc., Wilmington, DE.

TABLE 27b

| Number | Tangent Modulus of Elasticity in Bending<br>(ASTM D790-86) |                      |               |                             |
|--------|------------------------------------------------------------|----------------------|---------------|-----------------------------|
|        | Viscosity<br>(cp)                                          | Number of<br>Samples | Mean<br>(MPa) | Standard Deviation<br>(MPa) |
| 1      | 650                                                        | 5                    | 50.4          | 10.0                        |
| 2      | 220                                                        | 5                    | 79.0          | 8.3                         |
| 3      | 156                                                        | 5                    | 62.5          | 7.6                         |
| 4      | 1128                                                       | 5                    | 52.5          | 3.5                         |
| 5      | 258                                                        | 5                    | 86.5          | 9.2                         |
| 6      | 1085                                                       | 5                    | 57.9          | 8.9                         |

TABLE 27c

| Run Number | Flexural Strength (ASTM D790-86) |                  |                             |
|------------|----------------------------------|------------------|-----------------------------|
|            | Number of<br>Samples             | Mean<br>(MPa)    | Standard Deviation<br>(MPa) |
| 1          | 5                                | 1.2 <sup>1</sup> | 0.1                         |
| 2          | 5                                | 1.9 <sup>1</sup> | 0.1                         |
| 3          | 5                                | 1.2              | 0.1                         |
| 4          | 5                                | 1.6              | 0.1                         |
| 5          | 5                                | 2.1              | 0.2                         |
| 6          | 5                                | 1.0              | 0.1                         |

<sup>1</sup>Flexural Yield Strength

Example 28

Side chain crystallizable hydrocarbon polymer materials available as "VYBAR" 103 and "VYBAR" 253 from Petrolite Corporation, Tulsa, Okla., were blended with a hydrocarbon resin available as "REGALITE" R-91, from Hercules, Wilmington, Del. Stearic acid from J. T. Baker Inc. was added to the mixture. The materials were added in solid form to an aluminum tin and heated until molten and stirred in the amounts shown in Table 28a.

The blocking compositions of molten "VYBAR"/"REGALITE"/stearic acid blend was evaluated for viscosity as described in Example 3 except spindle no. 16 was used and the temperature was 70° C. The molten blends were poured into a mold, allowed to cool and solidify, and evaluated for Tangent Modulus of Elasticity in Bending and Flexural Strength as described in Example 26. The results are reported in Tables 28b and 28c.

TABLE 28a

| 5 | Run Number | Hydrocarbon Polymer 1 <sup>1</sup><br>(weight percent) | Hydrocarbon Polymer 2 <sup>2</sup><br>(weight percent) | Hydrocarbon Resin 1 <sup>3</sup><br>(weight percent) | Additive <sup>4</sup><br>(weight percent) |
|---|------------|--------------------------------------------------------|--------------------------------------------------------|------------------------------------------------------|-------------------------------------------|
|   | 1          | 17.5                                                   | 17.5                                                   | 60                                                   | 5                                         |

<sup>1</sup>Commercially available as VYBAR™ 103 from Petrolite, Tulsa, OK.<sup>2</sup>Commercially available as VYBAR™ 253 from Petrolite, Tulsa, OK.<sup>3</sup>Commercially available as REGALITE™ R-91 from Hercules, Inc., Wilmington, DE.<sup>4</sup>stearic acid (SA) available from J. T. Baker Inc.

TABLE 28b

| 15 | Tangent Modulus of Elasticity in Bending<br>(ASTM D790-86) |                   |                      |               |                             |
|----|------------------------------------------------------------|-------------------|----------------------|---------------|-----------------------------|
| 20 | Number                                                     | Viscosity<br>(cp) | Number of<br>Samples | Mean<br>(MPa) | Standard Deviation<br>(MPa) |
|    | 1                                                          | 792               | 5                    | 66.1          | 8.2                         |

TABLE 28c

| 25 | Flexural Strength (ASTM D790-86) |                      |               |                             |
|----|----------------------------------|----------------------|---------------|-----------------------------|
| 30 | Run Number                       | Number of<br>Samples | Mean<br>(MPa) | Standard Deviation<br>(MPa) |
|    | 1                                | 5                    | 1.6           | 0.1                         |

Example 29

Side chain crystallizable hydrocarbon polymer materials available as "VYBAR" 103 and "VYBAR" 253 from Petrolite Corporation, Tulsa, Okla., were blended with various hydrocarbon resins. The materials were added in solid form to an aluminum tin and heated until molten and stirred in the amounts shown in Table 29a.

The blocking compositions of molten "VYBAR"/hydrocarbon resin blends were evaluated for viscosity as described in Example 3 except spindle no. 16 was used and the temperature was 70° C. The molten blends were poured into a mold, allowed to cool and solidify, and evaluated for Tangent Modulus of Elasticity in Bending and Flexural Strength as described in Example 26. The results are reported in Tables 29b and 29c.

TABLE 29a

| 35 | Run Number | Hydrocarbon Polymer 1 <sup>1</sup><br>(weight percent) | Hydrocarbon Polymer 2 <sup>2</sup><br>(weight percent) | Hydrocarbon Resins<br>(weight percent) |
|----|------------|--------------------------------------------------------|--------------------------------------------------------|----------------------------------------|
|    | 1          | 18.4                                                   | 18.4                                                   | 63.2 <sup>3</sup>                      |
|    | 2          | 18.4                                                   | 18.4                                                   | 63.2 <sup>4</sup>                      |
|    | 3          | 18.4                                                   | 18.4                                                   | 63.2 <sup>5</sup>                      |

<sup>1</sup>Commercially available as VYBAR™ 103 from Petrolite, Tulsa, OK.<sup>2</sup>Commercially available as VYBAR™ 253 from Petrolite, Tulsa, OK.<sup>3</sup>PICCOTAC™ "B" from Hercules, Inc.<sup>4</sup>PICCOLYTE™ "HM90" from Hercules, Inc.<sup>5</sup>REGALREZ™ 1094 from Hercules, Inc.

TABLE 29b

| Run Number | Viscosity (cp) | Tangent Modulus of Elasticity in Bending (ASTM D790-86) |            |                          |
|------------|----------------|---------------------------------------------------------|------------|--------------------------|
|            |                | Number of Samples                                       | Mean (MPa) | Standard Deviation (MPa) |
| 1          | 4460           | 5                                                       | 153.9      | 106.6                    |
| 2          | 1552           | 5                                                       | 105.1      | 17.9                     |
| 3          | 2588           | 5                                                       | 113.3      | 22.8                     |

TABLE 29c

| Run Number | Flexural Strength (ASTM D790-86) |                  |                          |
|------------|----------------------------------|------------------|--------------------------|
|            | Number of Samples                | Mean (MPa)       | Standard Deviation (MPa) |
| 1          | 5                                | 3.7 <sup>1</sup> | 2.4                      |
| 2          | 5                                | 2.5 <sup>1</sup> | 0.3                      |
| 3          | 5                                | 2.8 <sup>1</sup> | 0.3                      |

<sup>1</sup>Flexural Yield Strength

Various modifications and alterations of this invention will be apparent to those skilled in the art without departing from the scope and spirit of this invention, and it should be understood that this invention is not limited to the illustrative embodiments set forth herein.

What is claimed is:

1. An ophthalmic lens block, comprising: a solidified mass of a thermoplastic blocking composition comprising a blend of between 30 and 65 weight percent of a hydrocarbon resin and between 20 and 70 weight percent of a side chain crystallizable hydrocarbon polymer or copolymer, the composition being solid at 21° C. and having a sufficiently low melting or softening point such that the composition may be placed adjacent to an ophthalmic lens blank while at its melting or softening point without damaging the lens blank.
  2. An ophthalmic lens block according to claim 1, wherein the hydrocarbon resin is selected from the group consisting of aliphatic resins, aromatic resins, mixed aliphatic/aromatic resins, hydrogenated pure aromatic resins, and hydrogenated mixed aromatic resins.
  3. An ophthalmic lens block according to claim 1, wherein the hydrocarbon resin is selected from the group consisting of aromatic resins, hydrogenated pure aromatic resins, and hydrogenated mixed aromatic resins, and wherein the hydrocarbon resin has a Ring and Ball Softening Point between about 70° and 110° C.
  4. An ophthalmic lens block according to claim 1, wherein the side chain crystallizable hydrocarbon polymer or copolymer is selected from the group consisting of ethylene polymers or copolymers having pendant hydrocarbon side chains of at least eight carbon atoms.
  5. An ophthalmic lens block according to claim 4, wherein the side chain crystallizable hydrocarbon polymer or copolymer has a Ring and Ball Softening Point between about 54° and 75° C.
  6. An ophthalmic lens block according to claim 4, wherein the side chain crystallizable hydrocarbon polymer or copolymer has a number average molecular weight between about 500 and 3,000.
  7. An ophthalmic lens block according to claim 1, wherein the thermoplastic blocking composition further comprises a modifier selected from the group consisting of: carboxylic acids of the general form  $\text{CH}_3(\text{CH}_2)_n\text{COOH}$ , where n is between about 10 and 16;
- 5
- 10
- 15
- 20
- 25
- 30
- 35
- 40
- 45
- 50
- 55
- 60
- 65
- 70
- 75
- 80
- 85
- 90

straight chain monohydric alcohols of the general form  $\text{CH}_3(\text{CH}_2)_n\text{OH}$ , where n is between about 11 and 19; and

branched chain monohydric alcohols having between 10 and 20 carbon atoms.

8. An ophthalmic lens block according to claim 7, wherein the blend comprises between 40 and 65 weight percent hydrocarbon resin, between 25 and 60 weight percent side chain crystallizable polymer or copolymer, and between 0.5 and 15 weight percent modifier.

9. An ophthalmic lens blocking kit, comprising a thermoplastic blocking composition according to claim 7; and

a lens blank tape or coating, wherein the blocking composition has sufficient adhesion to the lens blank tape or coating to hold an ophthalmic lens during a generating procedure.

10. An ophthalmic lens block according to claim 1, wherein the blend comprises between 40 and 65 weight percent hydrocarbon resin and between 25 and 60 weight percent side chain crystallizable polymer or copolymer.

11. An ophthalmic lens block according to claim 1, wherein the thermoplastic blocking composition has a melting or softening point between 45° and 75° C.

12. An ophthalmic lens block according to claim 1, wherein the solidified mass of a thermoplastic blocking composition has a mean flexural strength of at least 1 MPa at 21° C. and a mean bending modulus of at least 34.4 MPa at 21° C.

13. An ophthalmic lens block according to claim 1, wherein the block is formed entirely from the blocking composition.

14. An ophthalmic lens block according to claim 1, wherein the block comprises a preformed block defining a cavity with a lens blank, and wherein the cavity contains the solidified blocking composition.

15. An ophthalmic lens block according to claim 1, wherein the block comprises a preformed base block having a rear portion that is sized and adapted to fit the chuck of a lens processing machine, and a front portion having a negatively tapered peripheral edge and a curved front surface, wherein the front portion is adapted to mechanically retain the thermoplastic blocking composition to thereby form the lens block.

16. An ophthalmic lens blocking kit, comprising a thermoplastic blocking composition according to claim 1; and

a lens blank tape or coating, wherein the blocking composition has sufficient adhesion to the lens blank tape or coating to hold an ophthalmic lens during a generating procedure.

17. An ophthalmic lens block, comprising: a solidified mass of a thermoplastic blocking composition comprising a blend of

between 40 and 65 weight percent of a hydrocarbon resin selected from the group consisting of aliphatic resins, aromatic resins, mixed aliphatic/aromatic resins, hydrogenated pure aromatic resins, and hydrogenated mixed aromatic resins, wherein the hydrocarbon resin has a Ring and Ball Softening Point between about 70° and 110° C.;

between 25 and 60 weight percent of a side chain crystallizable hydrocarbon polymer or copolymer selected from the group consisting of ethylene polymers or copolymers having pendant hydrocarbon side chains of

**61**

at least eight carbon atoms, wherein the side chain crystallizable hydrocarbon polymer or copolymer has a Ring and Ball Softening Point between about 54° and 75° C.; and

between 2 and 10 weight percent of a modifier selected from the group consisting of carboxylic acids of the general form  $\text{CH}_3(\text{CH}_2)_n\text{COOH}$ , where n is between about 10 and 16, straight chain monohydric alcohols of the general form  $\text{CH}_3(\text{CH}_2)_n\text{OH}$ , where n is between about 11 and 19, and branched chain monohydric alcohols having between 10 and 20 carbon atoms, the composition being solid at 21° C. and having a sufficiently low melting or softening point such that the composition may be placed adjacent to an ophthalmic lens blank while at its melting or softening point without damaging the lens blank. <sup>5</sup>

**18.** An ophthalmic lens block according to claim 17, wherein the block comprises a preformed base block having a rear portion that is sized and adapted to fit the chuck of a lens processing machine, and a front portion having a negatively tapered peripheral edge and a curved front surface, wherein the front portion is adapted to mechanically retain the thermoplastic blocking composition to thereby form the lens block. <sup>15</sup>

**62**

**19.** An ophthalmic lens blocking kit, comprising a thermoplastic blocking composition according to claim 17; and

a lens blank tape or coating, wherein the blocking composition has sufficient adhesion to the lens blank tape or coating to hold an ophthalmic lens during a generating procedure.

**20.** An ophthalmic lens block, comprising: a solidified mass of a thermoplastic blocking composition comprising a blend of a hydrocarbon resin, a side chain crystallizable hydrocarbon polymer or copolymer, and a modifier selected from the group consisting of: carboxylic acids of the general form  $\text{CH}_3(\text{CH}_2)_n\text{COOH}$ , where n is between about 10 and 16; straight chain monohydric alcohols of the general form  $\text{CH}_3(\text{CH}_2)_n\text{OH}$ , where n is between about 11 and 19; and branched chain monohydric alcohols having between 10 and 20 carbon atoms, the composition being solid at 21° C. and having a sufficiently low melting or softening point such that the composition may be placed adjacent to an ophthalmic lens blank while at its melting or softening point without damaging the lens blank. <sup>10</sup>

\* \* \* \* \*